

# United States Patent Office

2,935,425

Patented May 3, 1960

1

2,935,425

## CHEMICAL NICKEL PLATING PROCESSES AND BATHS THEREFOR

Gregoire Gutzeit, Highland, Ind., Paul Talmey, Barrington, Ill., and Warren G. Lee, East Chicago, Ind., assignors to General American Transportation Corporation, Chicago, Ill., a corporation of New York

No Drawing. Application December 29, 1954  
Serial No. 478,492

29 Claims. (Cl. 117—130)

The present invention relates to improved processes of chemical nickel plating of catalytic materials employing baths of the nickel cation-hypophosphite anion type and to improved baths therefor, and more particularly to such processes and baths involving a continuous system of the character of that disclosed in U.S. Patent No. 2,658,839, granted on November 10, 1953, to Paul Talmey and William J. Crehan. This application is a continuation-in-part of the copending application of Gregoire Gutzeit, Paul Talmey and Warren G. Lee, Serial No. 376,968, filed August 27, 1953, now abandoned.

The chemical nickel plating of a catalytic material employing an aqueous bath of the nickel cation-hypophosphite anion type is based upon the catalytic reduction of nickel cations to metallic nickel and the corresponding oxidation of hypophosphite anions to phosphite anions with the evolution of hydrogen gas at the catalytic surface. The reactions take place when the body of catalytic material is immersed in the plating bath, and the exterior surface of the body of catalytic material is coated with nickel. The following elements are catalytic for the oxidation of hypophosphite anions and thus may be directly nickel plated: iron, cobalt, nickel, ruthenium, rhodium, palladium, osmium, iridium and platinum. The following elements are examples of materials which may be nickel plated by virtue of the initial displacement deposition of nickel thereon either directly or through a galvanic effect: copper, silver, gold, beryllium, germanium, aluminum, carbon, vanadium, molybdenum, tungsten, chromium, selenium, titanium and uranium. The following elements are examples of non-catalytic materials which ordinarily may not be nickel plated: bismuth, cadmium, tin, lead and zinc. The activity of the catalytic materials varies considerably and the following elements are particularly good catalysts in the chemical nickel plating bath: iron, cobalt, nickel and palladium. The chemical nickel plating process is auto-catalytic since both the original surface of the body being plated and the nickel metal that is deposited on the surface thereof are catalytic; and the reduction of the nickel cations to metallic nickel in the plating bath proceeds until all of the nickel cations have been reduced to metallic nickel, in the presence of an excess of hypophosphite anions, or until all of the hypophosphite anions have been oxidized to phosphite ions, in the presence of an excess of nickel cations.

In a batch plating process, the reactions are slowed-down rather rapidly as time proceeds because the anions, as contrasted with the cations, of the nickel salt that is dissolved in the plating bath combine with the hydrogen cations to form an acid, which, in turn, lowers the pH of the bath, and the reducing power of the hypophosphite anions is decreased as the pH value of the bath decreases. Moreover, there is a tendency for the early formation in the plating bath of a "black precipitate" that comprises a random chemical reduction of the nickel cations. Of course, this formation of the black precipitate comprises a decomposition of the plating bath,

2

and is particularly objectionable in that it causes the nickel deposit to be coarse, rough and frequently porous. Any fine solid particles suspended in the plating bath, or adhering to the walls of the plating vessel, at the plating temperature, initiate the formation of the black precipitate by acting as nuclei.

In a continuous plating process the reactions are maintained substantially at their initial rates by the regeneration of the plating bath, i.e., by the adding thereto of soluble nickel-containing and hypophosphite-containing reagents, as well as an alkali for pH control; however, the problem of preventing the formation of black precipitate in the plating bath and the consequent decomposition thereof is the same as that previously mentioned.

15 Moreover, another practical difficulty is encountered in the continuous plating process that is not encountered in the batch plating process in that there is a considerable build-up of the by-product phosphite therein as time proceeds and as a consequence of the cycling of the bath.

20 More particularly, while nickel hypophosphite is readily soluble in an aqueous solution, nickel phosphite is much less soluble in an aqueous solution; whereby there is a tendency, as the phosphite concentration of the plating bath builds up, for nickel phosphite to be precipitated therein, and thereby provide the solid particles that serve as nuclei for the formation of the black precipitate therein, previously mentioned. In passing it is noted that the initiation of the precipitation of nickel phosphite in the plating bath is indicated by turbidity thereof.

In carrying out the chemical nickel plating process on a commercial scale, the continuous system disclosed in the Talmey and Crehan patent mentioned may be employed; which system involves periodic or continuous regeneration of the plating bath by the addition thereto of appropriate ingredients for the purpose of maintaining substantially constant the composition of the bath as previously noted. More specifically in this system, there are provided a plating chamber and a reservoir; preferably one portion of the plating solution is stored at a relatively low temperature well below the boiling point thereof in the reservoir; and preferably another portion of the plating solution is held as a bath at a relatively high temperature slightly below the boiling point thereof in the plating chamber. The solution is continuously circulated at a low rate from the reservoir to the plating chamber and then back to the reservoir, the solution being heated substantially to the relatively high temperature after withdrawal thereof from the reservoir and before introduction thereof into the plating chamber, and the solution being cooled substantially to the relatively low temperature after withdrawal thereof from the plating chamber and before return thereof to the reservoir. The body that is to be nickel plated is immersed in the bath in the plating chamber and is subsequently withdrawn from the bath in the plating chamber after a time interval corresponding to the thickness of the nickel plating thereon that is desired; and during such time interval soluble reagents are added to the solution in the reservoir to maintain in the bath in the plating chamber during such time interval substantially the predetermined composition of the bath previously mentioned, so as to compensate for the ingredients of the bath that are exhausted during the time interval in the plating chamber. This regeneration of the solution in the reservoir consists essentially of adding thereto appropriate amounts of soluble nickel-containing and hypophosphite-containing reagents, as well as an alkali for pH control, as previously noted.

A typical chemical nickel plating bath that may be employed in the continuous process of the Talmey and Crehan patent is disclosed in U.S. Patent No. 2,658,841,

granted on November 10, 1953, to Gregoire Gutzeit and Abraham Krieg; which plating bath essentially comprises an aqueous acid solution of a nickel salt and a hypophosphite and a buffer in the form of an alkaline acetate; the pH of the bath being within the approximate range 4.5 to 5.6, the absolute concentration of hypophosphite ions in the bath being in the range 0.15 to 0.35 mole/liter, the ratio between nickel ions and hypophosphite ions in the bath being in the range 0.25 to 0.60, and the absolute concentration of acetate ions in the bath being approximately 0.120 mole/liter.

In the carrying out of the chemical nickel plating process on a commercial scale employing the continuous system of Talmey and Crehan, it has been discovered that the chemical nickel plating bath of Gutzeit and Krieg is not altogether satisfactory in that the bath does not have as fast a plating rate as is desirable; and moreover, the activity of the bath is within a relatively narrow pH range. Furthermore, nickel phosphite begins to precipitate at a phosphite ion concentration of about 0.07 mole/liter so that the stability of the bath is not that desired, and the useful life thereof is entirely too short.

The present invention is predicated upon the discovery that plating baths of the nickel cation-hypophosphite anion type mentioned may have their stable life increased, the plating rates thereof may be substantially increased, the useful life thereof may be greatly extended, and the activity thereof with regard to the usable pH range may be greatly broadened by the addition thereto of both a nickel chelating agent and an exalting additive. More particularly, the plating baths of the present invention have an increased stable life in that the ability thereof to hold nickel phosphite in solution at high phosphite concentrations is enhanced as evidenced by the clarity of the bath (the lack of turbidity thereof). Also, these plating baths have a nickel plating rate of at least 1 mil/hour (0.001"/hour) or expressed in c.g.s. units, of at least  $3.5 \times 10^{-4}$  gm./cm.<sup>2</sup>/min. Moreover, these plating baths have an activity within a broad pH range (4.0 to 11.0); and no precipitation of nickel phosphite takes place therein even at a phosphite ion concentration in some cases as high as 1.0 mole/liter. Further, the plating appearance on both metals and non-metals is excellent (bright, smooth and non-porous); and the adhesion of the nickel plating on both metallic and non-metallic bodies is excellent (no flaking of the nickel coating in bending, abrading and shock tests).

Specifically, the plating baths of the present invention consist essentially of an aqueous solution of a nickel salt and a hypophosphite and a nickel chelating agent and a separate and different exalting additive. The nickel chelating agent is selected from the group having the general formula:



where: R is an aliphatic radical, X is a functional group containing a dissociable hydrogen atom and selected from the class consisting of:



and Y is a functional group containing a negative atom acting as a center of coordination and selected from the class consisting of:



and wherein the functional groups X and Y are in alpha or beta positions to each other.

This group consists of saturated aliphatic hydroxycarboxylic acids and salts thereof, aminoalcohols, polyalcohols, aliphatic keto acids and salts thereof, aliphatic polyamines, aminocarbonyls, amine-oxydes, heteroaliphatic dicarboxylic acids and salts thereof, and short chain

aliphatic aminocarboxylic acids and salts thereof. The exalting additive is selected from the group consisting of simple short chain saturated aliphatic monocarboxylic acids including 3 to 5 carbon atoms and salts thereof.

5 simple short chain saturated aliphatic dicarboxylic acids including 3 to 6 carbon atoms and salts thereof, and short chain aliphatic aminocarboxylic acids and salts thereof.

Further, it is pointed out that the short chain aliphatic aminocarboxylic acids and salts thereof are named both 10 as chelating agents and as exalting additives since these compounds possess these two unrelated characteristics as explained more fully hereinafter.

In accordance with the process of the present invention, the chelating agent, if added in sufficient quantity, 15 substantially completely chelated all of the nickel ions in the plating bath, whereby it "ties-up" the nickel cations almost completely releasing only a small fraction thereof depending on the chelate stability constant (dissociation constant); whereas the exalting additive increases the

20 plating rate of the plating bath. Thus it will be understood that the plating bath, except for the exalting additive, would have an exceedingly low plating rate due to the tying-up of the nickel cations therein. However, this tying-up of the nickel cations in the plating bath is the

25 fundamental factor contributing to the clarity of the solution, preventing the formation of precipitated phosphites therein, and giving the bath an exceedingly long life in spite of the build-up of phosphite ions therein to a concentration even in excess of one molar. Of course, the

30 chelate of nickel in the plating bath must be water-soluble and of medium stability resulting in a bond strong enough to prevent the nickel ions from forming insoluble nickel compounds, such as the phosphite, the succinate, the malonate, etc., and mixed basic salts thereof, as explained

35 more fully hereinafter, but having a stability constant low enough to release the nickel cations required for the nickel plating operation permitting the exalting additive to bring about a plating rate of the bath of at least  $3.5 \times 10^{-4}$  gm./cm.<sup>2</sup>/min., as previously explained.

40 The general composition of a plating bath in accordance with the present invention essentially comprises an aqueous solution of a nickel salt and a hypophosphite (in addition to the nickel chelating agent and the exalting additive), as explained more fully hereinafter; whereby

45 the absolute concentration of hypophosphite anions in the bath is in the range 0.15 to 1.20 moles/liter, and the ratio between nickel cations and hypophosphite anions in the bath is in the range 0.25 to 1.60. The absolute concentration of the chelating agent in the bath is sufficient

50 to chelate at least 100% of the nickel cations therein, and the absolute concentration of the exalting additive in the bath is at least 0.04 mole/liter. In the plating bath, two separate additives for these two separate functions are employed. The pH of the bath is in the gen-

55 eral range 4.0 to 11.0, depending upon the particular ingredients of the bath, as explained more fully hereinafter; and the bath is utilized in the plating chamber of the continuous plating system at a temperature slightly below the boiling point thereof and above 90° C., ordi-

60 narily at about 97-99° C. The widening of the pH range is particularly desirable because adhesion of the plating to the base metal is improved at a low pH.

In view of the foregoing, it is the primary object of the present invention to provide an improved nickel plating process of the character described, in which the reactions involved are carried out more efficiently and under more stable conditions (clarity of solution) than heretofore, thereby rendering the process more desirable from a commercial standpoint.

65 70 Another object of the invention is to provide an improved aqueous chemical nickel plating bath that may be employed with advantage in the practice of the improved process.

Another object of the invention is to provide an improved nickel plating process of the character described,

that employs a plating bath of the nickel cation-hypophosphite anion type containing both a chelating agent and a separate and different exalting additive, wherein the chelating agent substantially completely chelates all of the nickel cations in the bath, and the exalting additive substantially increases the plating rate of the bath obtaining a plating rate thereof of at least  $3.5 \times 10^{-4}$  gm./cm.<sup>2</sup>/min.

A further object of the invention is to provide an improved nickel plating process of the continuous type involving an improved plating bath of the nickel cation-hypophosphite anion type so that the useful life thereof is greatly extended in that the plating bath remains clear notwithstanding the presence therein of a phosphite anion concentration as high as one molar.

A still further object of the invention is to provide an improved nickel plating bath of the character described that incorporates a novel combination of chelating agents and exalting additives.

These and other objects and advantages of the invention pertain to the particular arrangement of the steps of the process and of the composition of the plating bath, as will be understood from the foregoing and following description.

In accordance with the process of the present invention, the article to be nickel plated and normally having a catalytic surface is properly prepared by mechanical cleaning, degreasing and light pickling substantially in accordance with standard practices in electroplating processes. For example, in the nickel plating of a steel object, it is customary to clean the rust and mill scale from the object, to degrease the object, and then lightly to pickle the object in a suitable acid, such as hydrochloric acid. The object is then immersed in a suitable volume of the bath containing the proper proportions of nickel cations, hypophosphite anions, chelating agent and exalting additive, the pH of the bath having been, if necessary, adjusted to an optimum value by the addition of an appropriate acid or base, and the bath having been heated to a temperature just below its boiling point, such as 99° C., at atmospheric pressure. Almost immediately hydrogen bubbles are formed on the catalytic surface of the steel object and escape in a steady stream from the bath while the surface of the steel object is slowly coated with metallic nickel (containing some phosphorus). The steel object is ultimately removed from the bath after an appropriate time interval corresponding to the required thickness of the nickel coating deposited thereon that is desired. Ultimately the steel object is rinsed off with water, and is then ready for use.

With respect to the composition of the bath, it essentially comprises an aqueous solution containing nickel cations, hypophosphite anions, a chelating agent and an exalting additive, as previously noted. For example, the nickel cations may be derived from the nickel chloride, nickel sulfate, etc., and the hypophosphite anions may be derived from sodium, potassium, etc., hypophosphites or various combinations thereof. The chelating agent and the exalting additive are introduced into the bath normally as the acids or as the soluble salts thereof, etc.; and the desired pH of the bath is established by the eventual introduction thereinto of hydrochloric acid or a weak alkali, such as sodium bicarbonate.

The terms "cation," "anion" and "ion" as employed herein, except where specifically noted, include the total quantity of the corresponding elements that are present in the plating bath, i.e., both undissociated and dissociated material. In other words 100% dissociation is assumed when the terms noted are used in connection with molar ratios and concentrations in the plating bath. Also hereinafter the expression "percent exaltation" is employed with the arbitrary definition as the percent increase in the rate of hydrogen evolution with reference to a given hypophosphite solution resulting from the addition thereto of the exalting additive.

Turning now more particularly to the introduction of the nickel chelating agent into the bath, the following examples of saturated aliphatic hydroxy-carboxylic acids have been found to be particularly suitable:

5 Hydroxyacetic acid (glycollic acid)



10 Monohydroxysuccinic acid (malic acid)



15 Dihydroxysuccinic acid (tartaric acid)



20 Gluconic acid



25 Citric acid



30 Hydroxymalonic acid



35 Trihydroxyglutaric acid



40 Alpha-hydroxypropionic acid (lactic acid)



45 Beta-hydroxypropionic acid



50 1-beta-hydroxybutyric acid



55 As a matter of convenience, the salts of the saturated aliphatic hydroxycarboxylic acids mentioned, particularly the alkali salts thereof, may be employed in the preparation of the plating bath, since the alkali salts of these acids are usually more readily obtainable upon the market.

60 The following aminoalcohol has been found to be particularly suitable:

65 2-aminoethanol



70 The following polyalcohols have been found to be particularly suitable:

75 Trihydroxyalcohol (glycerol)



## Hexahydroxyalcohol (mannitol)



The following aliphatic keto-acids have been found to be particularly suitable:

## Pyruvic acid



## Levulinic acid



Of course the salts of these aliphatic keto acids, particularly the alkali salts thereof, may be employed.

The following aliphatic polyamines have been found to be suitable:

## Trimethylamine



## Propylenediamine



The following aminocarbonyl and amine-oxyde have been found to be suitable:

## Semi-carbazide



## Diethylene-imide-oxyde (morpholine)



The following heteroaliphatic dicarboxylic acid has been found to be particularly suitable:

## Diglycollic acid



Of course, the salts of this heteroaliphatic dicarboxylic acid, particularly the alkali salts thereof, may be employed.

The following aliphatic amino-acids have been found to be particularly suitable:

## Aminoacetic acid (glycine)



## Alpha-aminopropionic acid (alpha-alanine)



## Beta-aminopropionic acid (beta-alanine)



## Alpha-aminobutyric acid



## Aminosuccinic acid (aspartic acid)



## Iminodiacetic acid



## Iminotriacetic acid



## Ethylenediaminetetraacetic acid



Of course, the salts of the amino-acids, particularly the alkali salts thereof, may be employed.

Turning now more particularly to the introduction of the exalting additive into the bath, the previously-mentioned short chain aliphatic aminocarboxylic acids and salts thereof are also particularly suitable as exalting additives.

Furthermore, the following simple short chain saturated aliphatic dicarboxylic acids including 3 to 6 carbon atoms have been found to be particularly useful as exalting additives:

## Malonic acid



## Succinic acid



## Glutaric acid



## Adipic acid



Of course, the salts of the simple short chain saturated aliphatic dicarboxylic acids, particularly the alkali salts thereof, may be employed.

The following simple short chain saturated aliphatic monocarboxylic acids including 3 to 5 carbon atoms have been found to be particularly useful as exalting additives:

## Propionic acid



## Butyric acid



## Valeric acid



Of course, the salts of these simple short chain saturated aliphatic monocarboxylic acids, particularly the alkali salts thereof, may be employed.

As previously noted, the chelating agent mentioned above form water-soluble chelates with the nickel ions in the plating bath, which chelates in the cases of the hydroxycarboxylic acids and the aminocarboxylic acids may be either alpha or beta position respectively forming five-membered or six-membered chelate rings as follows:

(1)



(2)



(3)



(4)



As previously noted, the stability of the water-soluble nickel chelates formed in the bath by the chelating additives are variable and the order of stability of some of the nickel chelates produced by some of the hydroxy-acids is approximately as follows (from the more stable to the less stable): tartaric acid, malic acid, gluconic acid, citric acid, glycolic acid. An important factor that enters into nickel chelate formation by hydroxy-acids is the pH of the solution; for instance, the following pH values represent the range in which the chelate of nickel with three hydroxy-acids is stable (i.e., where no nickel phosphite or basic salts are precipitated in the presence of 0.30 mole/liter of nickel phosphite over a range from room temperature to 100° C.):

Citric acid ..... pH 4.6 to 4.8 and 6.5 to 11.0.  
 Malic acid ..... pH 4.5 to 5.7.  
 Tartaric acid ..... pH 4.5 to 5.0.

For the purpose of studying the increase of the hydrogen gas evolution due to exaltation with the use of different additives including those involved in the discovery of the present invention, i.e., simple short chain saturated aliphatic dicarboxylic acids and aliphatic aminocarboxylic additives, and other additives which have been used or suggested for chemical nickel plating baths, tests were made with test solutions of 50 cc. and containing sodium hypophosphite at a concentration of 0.225 mole/liter (to which a trace of nickel salt, i.e. 0.0024 mole/liter, was added to initiate the reaction at a vigorous rate). Pickled pieces of mild steel, 20 cm.<sup>2</sup> area, were introduced for periods of 30 minutes each. The different test solutions respectively contain no additive, and additives in the form of salts of the following acids: formic, acetic, propionic, butyric, valeric, malonic, succinic, glutaric, tartaric, citric, hydroxypropionic, aminoacetic and aspartic.

Specifically the additives, when used, were employed as the sodium salts of the corresponding acids at a concentration of 0.125 mole/liter of the anion; and the hydrogen gas evolved was collected and its volume measured by the usual methods.

The exaltation test results were as follows:

|    | Additive (Anion) 0.125 moles/l. | H <sub>2</sub> evolved in 30 min. from 50 cc. solution at 0.225 moles/l. sodium hypophosphite at 98° C. | Percent Exaltation |
|----|---------------------------------|---------------------------------------------------------------------------------------------------------|--------------------|
| 5  | None                            | 80                                                                                                      | 0                  |
|    | Formic                          | 85                                                                                                      | 6                  |
|    | Acetic                          | 155                                                                                                     | 94                 |
| 10 | Propionic                       | 190                                                                                                     | 136                |
|    | Butyric                         | 180                                                                                                     | 125                |
|    | Valeric                         | 170                                                                                                     | 113                |
|    | Malonic                         | 250                                                                                                     | 213                |
|    | Succinic                        | 220                                                                                                     | 175                |
|    | Glutaric                        | 210                                                                                                     | 163                |
|    | Tartaric                        | 100                                                                                                     | 32                 |
| 15 | Citric                          | 130                                                                                                     | 63                 |
|    | Hydroxypropionic                | 145                                                                                                     | 81                 |
|    | Aminoacetic                     | 180                                                                                                     | 125                |
|    | Aspartic                        | 250                                                                                                     | 213                |

From these exaltation tests, it will be observed that the following anions give exaltation values over 100% (which appears to be the lower limit of practical efficiency): propionic, butyric, valeric, malonic, succinic, glutaric, aminoacetic, aspartic.

As a practical matter, it has been discovered that the soluble propionates, succinates and aminoacetates are the most suitable as they are cheap, readily obtainable upon the market in commercial quantities and produce the desired exaltation to a satisfactory degree.

In the formulation of plating baths in accordance with the present invention, at least 100% of the nickel cations should be chelated so that the ratio of the hydroxy-acid/Ni<sup>++</sup> is at least two for monobasic and dibasic hydroxy-acids, and at least one for tribasic hydroxy-acids.

In the use of short chain aliphatic aminocarboxylic acids, simple short chain saturated aliphatic dicarboxylic acids and simple short chain saturated aliphatic monocarboxylic acids, it is believed that this phenomenon results from the formation of heteropoly-acids between the organic additive and the hypophosphite anions which compete with the nickel chelate formation. Thus if the nickel chelate is too stable, insufficient nickel cations are available for deposition and the plating rate becomes low despite the exalting effect produced by the organic additive.

The composite chelating effect and exalting effect of the various chelating agents and exalting additives in the plating baths were established by a series of plating tests that were made employing a series of test-plating baths of the general character of those previously described and as set forth more particularly hereinafter.

In the various plating tests appearing hereinafter weights of nickel plating deposited are reported in gms., and plating rates are usually reported in gm./cm.<sup>2</sup>/min. although occasionally plating rates are reported in mils/hour (i.e. 0.001"/hour).

In a plating bath of the character noted, substantially complete chelating of the nickel ions maintains a clear plating solution but results in a low and impractical plating rate; whereas the addition of an exaltant to the chelating bath will raise the plating rate thereof to a practical value as indicated by the following tests involving Baths A, B, C, D, E, F and G, having the specific compositions indicated hereinafter.

A simple aqueous malic acid plating bath was first prepared that had the following composition:

|    | Bath A:              | M.p.l. |
|----|----------------------|--------|
| 70 | Nickel chloride      | 0.0675 |
|    | Sodium hypophosphite | 0.225  |
|    | Malic acid           | 0.0675 |

The pH value was adjusted with NaOH and HCl.

Utilizing this plating bath, properly cleaned steel samples of 20 cm.<sup>2</sup> area were plated for 10 minutes, the

volume of the bath being 50 cc. and the temperature thereof being about 98° C., with the following results:

|                                     |       |       |
|-------------------------------------|-------|-------|
| Initial pH.....                     | 4.50  | 5.02  |
| Final pH.....                       | 4.16  | 4.35  |
| Wt. gain.....                       | 0.057 | 0.706 |
| Plating rate, R $\times 10^4$ ..... | 2.85  | 3.53  |

To the Bath A, there was added 0.06 m.p.l. of sodium succinate, as exaltant, in order to produce the Bath B, and the plating tests were repeated under otherwise identical conditions, with the following results:

|                                     |        |        |
|-------------------------------------|--------|--------|
| Initial pH.....                     | 4.50   | 5.10   |
| Final pH.....                       | 4.00   | 4.48   |
| Wt. gain.....                       | 0.0701 | 0.0853 |
| Plating rate, R $\times 10^4$ ..... | 3.51   | 4.28   |

From a comparison of the plating tests using the Baths A and B, it will be observed that the plating rates are substantially exalted by the addition of the small amount of sodium succinate mentioned, the plating rate of Bath B at the higher pH being very satisfactory.

Then a simple aqueous 2-aminoethanol plating bath was first prepared that had the following composition:

Bath C:

|                                         |               |
|-----------------------------------------|---------------|
| Nickel chloride .....                   | m.p.l. 0.0675 |
| Sodium hypophosphite .....              | m.p.l. 0.225  |
| 2-aminoethanol .....                    | m.p.l. 0.135  |
| Stabilizing ion: Pb <sup>++</sup> ..... | p.p.m. 1      |

The pH value was adjusted with HC1.

Utilizing this plating bath, properly cleaned steel samples of 20 cm.<sup>2</sup> area were plated for 10 minutes, the volume of the bath being 50 cc. and the temperature thereof being about 98° C., with the following results:

|                                    |      |
|------------------------------------|------|
| Initial pH .....                   | 4.50 |
| Final pH .....                     | 2.54 |
| Weight gain .....                  | 0.01 |
| Plating rate R $\times 10^4$ ..... | 0.50 |

To the Bath C, there was added 0.09 m.p.l. of sodium succinate as exaltant in order to produce the Bath D, and the plating tests were repeated under otherwise identical conditions, with the following results:

|                                    |        |
|------------------------------------|--------|
| Initial pH .....                   | 4.45   |
| Final pH .....                     | 4.08   |
| Weight gain .....                  | 0.0760 |
| Plating rate R $\times 10^4$ ..... | 3.80   |

From a comparison of the plating tests using the Baths C and D, it will be observed that the plating rate is roughly 7 times higher after the addition of the exaltant. In passing, it is noted that the pH values given in these tests are not optimum but were chosen only for comparison purposes.

Then in a simple aqueous hydroxyacetic acid plating bath was first prepared that had the following composition:

Bath E:

|                            |              |
|----------------------------|--------------|
| Nickel chloride .....      | m.p.l. 0.126 |
| Sodium hypophosphite ..... | m.p.l. 0.094 |
| Hydroxyacetic acid .....   | m.p.l. 0.092 |
| pH .....                   | 4.6          |

Utilizing this plating bath, a properly cleaned steel sample of 20 cm.<sup>2</sup> area was plated for 10 minutes, the volume of the bath being 50 cc. and the temperature thereof being about 99° C., and the plating rate was 1.84 $\times 10^{-4}$  gm./cm.<sup>2</sup>/min.

To the Bath E, there was added 0.06 m.p.l. of sodium succinate as exaltant in order to produce the Bath F, and the plating test was repeated under otherwise identical

conditions and there was obtained a plating rate of 3.43 $\times 10^{-4}$  gm./cm.<sup>2</sup>/min.

From a comparison of the plating tests using the Baths E and F, it will be observed that the plating rate is substantially exalted by the addition of the small amount of sodium succinate mentioned.

For the purpose of demonstrating that this improvement in the plating rate of the Bath F over the Bath E is not due merely to the increased concentration of an organic additive, an additional aqueous bath was employed having the following composition:

Bath G:

|                                         |              |
|-----------------------------------------|--------------|
| Nickel chloride .....                   | m.p.l. 0.126 |
| Sodium hypophosphite .....              | m.p.l. 0.094 |
| Hydroxyacetic acid .....                | m.p.l. 0.152 |
| Stabilizing ion: Pb <sup>++</sup> ..... | p.p.m. 1.0   |

It is noted that the Bath G contains no exaltant but an additional quantity of 0.06 m.p.l. of hydroxyacetic acid over that of the Bath F, so that the Baths F and G contain the same concentration of organic additive.

Utilizing this plating bath, a properly cleaned steel sample of 20 cm.<sup>2</sup> area was plated for 10 minutes, the volume of the bath being 50 cc. and the temperature thereof being about 99° C., and the plating rate was: 1.80 $\times 10^{-4}$  gm./cm.<sup>2</sup>/min.

From a comparison of the plating tests using the Baths F and G, it will be observed that the higher plating rate of the Bath F is due to the exalting additive and not to the total concentration of organic ion present.

A series of plating tests were then conducted demonstrating that the various complexing agents, properly selected as to the obtained stability coefficient, in amounts sufficient to give substantially complete chelation, and used with the addition of an exalting additive, result in chemical plating baths having high rates of deposition.

In a series of these plating tests a number of aqueous baths having the particular compositions indicated below were employed in the plating of properly cleaned steel samples of 20 cm.<sup>2</sup> area, the volume of the bath being 50 cc. and the temperature thereof being about 99° C., with the following results:

| Bath Compositions             | Initial pH    | Rate (gm./cm. <sup>2</sup> /min. $\times 10^4$ , 10 minutes) |       |
|-------------------------------|---------------|--------------------------------------------------------------|-------|
|                               |               | No. 1                                                        | No. 2 |
| No. 1<br>Malic acid .....     | 5.10          | 4.60                                                         |       |
| Sodium succinate .....        | m.p.l. 0.16   |                                                              |       |
| Sodium hypophosphite .....    | m.p.l. 0.06   |                                                              |       |
| Nickel sulfate .....          | m.p.l. 0.225  |                                                              |       |
| No. 2<br>Sodium citrate ..... | 6.90          | 4.68                                                         |       |
| Sodium succinate .....        | m.p.l. 0.09   |                                                              |       |
| Sodium hypophosphite .....    | m.p.l. 0.225  |                                                              |       |
| Nickel sulfate .....          | m.p.l. 0.0675 |                                                              |       |
| No. 3<br>Sodium citrate ..... | 7.50          | 5.41                                                         |       |
| Sodium aminoacetate .....     | m.p.l. 0.045  |                                                              |       |
| Diglycolic acid .....         | m.p.l. 0.09   |                                                              |       |
| Sodium hypophosphite .....    | m.p.l. 0.225  |                                                              |       |
| Nickel chloride .....         | m.p.l. 0.09   |                                                              |       |
| No. 4<br>Sodium citrate ..... | 7.50          | 5.41                                                         |       |
| Sodium aminoacetate .....     | m.p.l. 0.045  |                                                              |       |
| Sodium succinate .....        | m.p.l. 0.09   |                                                              |       |
| Sodium hypophosphite .....    | m.p.l. 0.225  |                                                              |       |
| Nickel sulfate .....          | m.p.l. 0.09   |                                                              |       |

Employing the Bath No. 2 (citrate-succinate), it was found that the effect of pH variations is as follows:

| pH        | 10 min. Plating Rate (gm./cm. <sup>2</sup> /min. $\times 10^4$ ) |
|-----------|------------------------------------------------------------------|
| 4.50..... | 2.65.....                                                        |
| 5.00..... | 3.50—Fair.                                                       |
| 5.50..... | 3.56—Fair.                                                       |
| 6.00..... | 4.68—Good.                                                       |
| 7.65..... | 4.71—Good.                                                       |
| 7.85..... | 4.50—Good.                                                       |

Employing the Bath No. 4 (citrate-aminoacetate-succinate) it was found that the effect of pH variations is as follows:

| pH   | 10 min. Plating Rate<br>(gm./cm. <sup>2</sup> /min. $\times 10^4$ ) |
|------|---------------------------------------------------------------------|
| 7.00 | 3.91—good.                                                          |
| 7.50 | 5.41—very good.                                                     |
| 8.00 | 5.55—very good.                                                     |
| 8.50 | 5.73—very good.                                                     |
| 9.00 | 5.95—very good.                                                     |

In view of the foregoing, it is apparent that the Baths Nos. 2 and 4, are most effective in the alkaline range. With certain basic metals, as for instance aluminum, a high pH is desirable.

In another series of these plating tests a number of aqueous baths having the particular compositions indicated below were employed:

Bath compositions:

M.p.l.

|                                |       |
|--------------------------------|-------|
| No. 5—                         |       |
| Hydroxyacetic (glycollic acid) | 0.18  |
| Sodium succinate               | 0.06  |
| Nickel sulfate                 | 0.09  |
| Sodium hypophosphite           | 0.225 |
| No. 6—                         |       |
| Lactic acid                    | 0.18  |
| Sodium succinate               | 0.06  |
| Nickel sulfate                 | 0.09  |
| Sodium hypophosphite           | 0.225 |
| No. 7—                         |       |
| Malic acid                     | 0.16  |
| Sodium succinate               | 0.06  |
| Nickel sulfate                 | 0.09  |
| Sodium hypophosphite           | 0.225 |
| No. 8—                         |       |
| Tartaric acid                  | 0.16  |
| Sodium succinate               | 0.06  |
| Nickel sulfate                 | 0.09  |
| Sodium hypophosphite           | 0.225 |
| No. 9—                         |       |
| Sodium citrate                 | 0.05  |
| Sodium succinate               | 0.06  |
| Nickel sulfate                 | 0.09  |
| Sodium hypophosphite           | 0.225 |

Utilizing these plating baths properly cleaned steel samples of 20 cm.<sup>2</sup> area were plated for 10 minutes, the volume of the bath being 50 cc. and the temperature thereof being about 99° C., with the following results:

| Bath No.                     | 5      | 6      | 7      | 8      | 9      |
|------------------------------|--------|--------|--------|--------|--------|
| Initial pH                   | 4.65   | 4.75   | 5.10   | 4.75   | 6.90   |
| Final pH                     | 4.05   | 4.05   | 4.60   | 4.23   | 4.90   |
| Wt. Gain                     | 0.0908 | 0.1057 | 0.0916 | 0.0617 | 0.0937 |
| Plating rate $R \times 10^4$ | 4.55   | 5.30   | 4.58   | 3.09   | 4.68   |

From the foregoing, it will be observed that the Bath No. 6 (lactic acid-succinate) produces the highest plating rate, while the Bath No. 8 (tartaric acid-succinate) produces the lowest plating rate. This is due to the fact that the lactic acid nickel chelate is least stable, while the tartaric acid nickel chelate is most stable. When 0.3 m.p.l. of phosphite ion is added to these baths precipitation of nickel phosphite takes place in the Bath No. 6 (lactic acid-succinate), whereby the Baths Nos. 5, 7 and 9 are preferred in the continuous plating system, while the Bath No. 6 may be used advantageously for batch plating.

In another series of these plating tests an aqueous bath having the particular composition indicated below was employed:

Bath composition:

No. 10—

|                                                         |   |        |        |
|---------------------------------------------------------|---|--------|--------|
| Sodium citrate                                          | — | m.p.l. | 0.05   |
| Sodium succinate                                        | — | m.p.l. | 0.06   |
| Nickel sulfate                                          | — | m.p.l. | 0.0675 |
| Sodium hypophosphite                                    | — | m.p.l. | 0.225  |
| Ratios:                                                 |   |        |        |
| Ni <sup>++</sup> /hypo <sup>-</sup>                     | — | 0.33   |        |
| Hydroxy-acid/Ni <sup>++</sup>                           | — | 2.00   |        |
| Initial pH adjusted with sulfuric acid or caustic soda. |   |        |        |

Utilizing this plating bath properly cleaned steel samples of 20 cm.<sup>2</sup> area were plated for 10 minutes, the volume of the bath being 50 cc. and the temperature thereof being about 99° C., with the following results (averages of duplicate tests being reported):

| Initial pH            | 4.5    | 4.5    | 5.0    | 5.0    | 5.5    |
|-----------------------|--------|--------|--------|--------|--------|
| Final pH              | 3.95   | 3.95   | 4.32   | 4.32   | 4.30   |
| Weight gain           | 0.0531 | 0.0526 | 0.0707 | 0.0691 | 0.0717 |
| Rate, $R \times 10^4$ | 2.66   | 2.63   | 3.54   | 3.46   | 3.58   |
| Initial pH            | 5.5    | 7.65   | 7.65   | 7.95   | 7.95   |
| Final pH              | 4.30   | 5.0    | 5.0    | 5.22   | 5.22   |
| Weight gain           | 0.0706 | 0.0940 | 0.0941 | 0.0925 | 0.0873 |
| Rate, $R \times 10^4$ | 3.58   | 4.70   | 4.71   | 4.63   | 4.37   |

In view of the foregoing it is apparent that the Bath No. 10 (citrate-succinate) is most effective at a pH of around 7.50.

The Bath No. 10 was slightly modified by varying the sodium succinate content to provide three different batches thereof having the following compositions:

| Bath No. 10...       | Batch Compositions |        |        |
|----------------------|--------------------|--------|--------|
|                      | I                  | II     | III    |
| Sodium citrate       | M.p.l.             | M.p.l. | M.p.l. |
| Sodium succinate     | 0.05               | 0.05   | 0.05   |
| Nickel sulfate       | 0.02               | 0.04   | 0.06   |
| Sodium hypophosphite | 0.0675             | 0.0675 | 0.0675 |
|                      | 0.225              | 0.225  | 0.225  |

Employing these batches of the Bath No. 10 properly cleaned steel samples of 20 cm.<sup>2</sup> area were plated in duplicate tests for 10 minutes, the temperature of the bath being about 98° C., with the following results:

| Batches of Bath No. 10 | I      | I      | II     | II     | III    | III    |
|------------------------|--------|--------|--------|--------|--------|--------|
| Sodium succinate       | 0.02   | 0.02   | 0.04   | 0.04   | 0.06   | 0.06   |
| Initial pH             | 7.30   | 7.30   | 7.30   | 7.30   | 7.65   | 7.65   |
| Final pH               | 6.60   | 6.60   | 6.40   | 6.40   | 5.0    | 5.0    |
| Wt. Gain               | 0.0772 | 0.0756 | 0.0913 | 0.0906 | 0.0940 | 0.0941 |
| Rate, $R \times 10^4$  | 3.86   | 3.78   | 4.57   | 4.53   | 4.70   | 4.71   |

In view of the foregoing, it will be observed that the Batch III of the Bath No. 10 (citrate-succinate) yields the highest plating rate employing 0.06 mole/liter of sodium succinate.

In another series of these plating tests, an aqueous bath having the particular composition indicated below was employed:

Bath composition:

No. 11—

|                                                              |   |        |        |
|--------------------------------------------------------------|---|--------|--------|
| Malic acid                                                   | — | m.p.l. | 0.135  |
| Sodium succinate                                             | — | m.p.l. | 0.06   |
| Nickel chloride                                              | — | m.p.l. | 0.0675 |
| Sodium hypophosphite                                         | — | m.p.l. | 0.225  |
| Ratios:                                                      |   |        |        |
| Ni <sup>++</sup> /hypo <sup>-</sup>                          | — | 0.33   |        |
| Hydroxy-acid/Ni <sup>++</sup>                                | — | 2.00   |        |
| Initial pH adjusted with caustic soda and hydrochloric acid. |   |        |        |

## 15

Utilizing this plating bath properly cleaned steel samples of 20 cm.<sup>2</sup> area were plated for 10 minutes and 60 minutes, the volume of the bath being 50 cc. and the temperature thereof being 99° C. with the following results:

|                                                   |        |        |        |        |        |
|---------------------------------------------------|--------|--------|--------|--------|--------|
| Initial pH.....                                   | 4.5    | 5.0    | 5.5    | 6.0    | 7.1    |
| Plating rate (10 min. test) R $\times 10^4$ ..... | 3.51   | 4.27   | 4.72   | 4.80   | 4.91   |
| Wt. gain in (60 min.).....                        | 0.1851 | 0.1866 | 0.1880 | 0.1885 | 0.1896 |

The optimum pH for the Bath No. 11 is around neutrality; and in the alkaline range this plating bath has a tendency to gel.

Another series of plating tests were run for 10 minutes and 60 minutes employing the Bath No. 11, at variable pH upon properly cleaned steel samples of 20 cm.<sup>2</sup> area, the volume of the bath being 50 cc. and the temperature thereof being about 99° C., with the following results:

|                                    |        |        |        |        |        |        |        |
|------------------------------------|--------|--------|--------|--------|--------|--------|--------|
| Time of test.....                  | 10     | 60     | 10     | 60     | 10     | 60     | 10     |
| Initial pH.....                    | 4.50   | 4.50   | 5.10   | 5.10   | 6.00   | 6.00   | 7.10   |
| Wt. gain.....                      | 0.0701 | 0.1851 | 0.0853 | 0.1866 | 0.0981 | 0.1893 | 0.0981 |
| Plating rate R $\times 10^4$ ..... | 3.51   | -----  | 4.28   | -----  | 4.81   | -----  | 4.91   |

In conjunction with these tests, it is noted that at about pH 7.0 the plating rate is almost  $5.0 \times 10^{-4}$  gm./cm.<sup>2</sup>/min., i.e. over 1.4 mils/hour.

In passing, it is noted that the optimum pH, which is around 4.6 for a succinate bath (without malic acid) shifts toward the neutral point in a bath containing all the nickel cations in the form of a chelate. As will be seen hereinafter the contrary is true when an amino-acid is used as the chelating agent in conjunction with succinate as the exalting additive.

In order to determine the effect of increased succinate concentrations two additional substantially identical plating tests were run at pH 5.5, one with the Bath No. 11 containing sodium succinate at a concentration of 0.06 m.p.l., and another with an otherwise identical bath (No. 12) containing sodium succinate at a concentration of 0.12 m.p.l., with the following results:

| Bath Compositions                                 | No. 11 | No. 12 |
|---------------------------------------------------|--------|--------|
| Sodium succinate (m.p.l.).....                    | 0.06   | 0.12   |
| Initial pH.....                                   | 5.5    | 5.5    |
| Plating rate (10 min. test) R $\times 10^4$ ..... | 4.73   | 5.12   |

A continuous plating test was conducted utilizing the Bath No. 12 containing sodium succinate at a concentration of 0.12 m.p.l., as previously noted; and a plating rate of  $5.09 \times 10^{-4}$  gm./cm.<sup>2</sup>/min. was achieved.

In another series of these plating tests, an aqueous bath having the particular composition indicated below was employed:

## Bath composition:

## Bath No. 13—

|                            |        |       |
|----------------------------|--------|-------|
| Malic acid .....           | m.p.l. | 0.18  |
| Sodium succinate .....     | m.p.l. | 0.06  |
| Nickel chloride .....      | m.p.l. | 0.09  |
| Sodium hypophosphite ..... | m.p.l. | 0.225 |

## Ratios:

|                                           |      |
|-------------------------------------------|------|
| Ni <sup>++</sup> /hypo <sup>-</sup> ..... | 0.40 |
| Hydroxy-acid/Ni <sup>++</sup> .....       | 2.0  |

Utilizing this plating bath, properly cleaned steel samples of 20 cm.<sup>2</sup> area were plated for 10 minutes and 60 minutes, the volume of the bath being 50 cc. and the temperature thereof being about 99° C., with the following results:

|                                                   |        |        |        |
|---------------------------------------------------|--------|--------|--------|
| Initial pH.....                                   | 4.50   | 5.00   | 5.50   |
| Plating rate (10 min. test) R $\times 10^4$ ..... | 3.82   | 4.58   | 4.47   |
| Wt. gain in 60 min.....                           | 0.2130 | 0.2210 | 0.2227 |

## 16

Comparing the Baths Nos. 11, 12 and 13, it will be observed that plating rates and 60 minute nickel deposits are greater employing the Bath No. 13 utilizing a Ni<sup>++</sup>/hypo<sup>-</sup> ratio of 0.4 rather than the ratio 0.33 as in the Baths Nos. 11 and 12.

In another of these plating tests, an aqueous bath having the particular composition indicated below was employed:

## 10 Bath composition:

## Bath No. 14—

|                            |        |       |
|----------------------------|--------|-------|
| Sodium citrate .....       | m.p.l. | 0.045 |
| Aminoacetic acid .....     | m.p.l. | 0.18  |
| Nickel chloride .....      | m.p.l. | 0.09  |
| Sodium hypophosphite ..... | m.p.l. | 0.225 |

## Ratios:

|                                           |     |
|-------------------------------------------|-----|
| Ni <sup>++</sup> /hypo <sup>-</sup> ..... | 0.4 |
| Tribasic hydroxy-acid/Ni .....            | 0.5 |

## 30 Stabilizing ions:

|                        |        |   |
|------------------------|--------|---|
| Pb <sup>++</sup> ..... | p.p.m. | 1 |
| Te <sup>++</sup> ..... | p.p.m. | 1 |

Initial pH adjusted with HCl and NaOH.

Utilizing this plating bath properly cleaned steel samples of 60 cm.<sup>2</sup> area were plated. The bath was employed in a continuous plating system having a plating chamber volume of 300 cc., the volume of the bath being 2 liters and the temperature thereof being about 99° C.; and the following results were obtained:

|                                    |        |
|------------------------------------|--------|
| Initial pH .....                   | 6.60   |
| Final pH .....                     | 6.35   |
| Weight gain .....                  | 1.1245 |
| Rate R $\times 10^4$ .....         | 5.21   |
| Duration of test, min. .....       | 36     |
| Flow rate solution, cc./min. ..... | 55.5   |

45 In another of these plating tests, an aqueous bath having the particular composition indicated below was employed:

## Bath composition:

## Bath No. 15—

|                        |        |       |
|------------------------|--------|-------|
| Sodium citrate .....   | m.p.l. | 0.045 |
| Malic acid .....       | m.p.l. | 0.09  |
| Sodium succinate ..... | m.p.l. | 0.06  |
| Nickel chloride .....  | m.p.l. | 0.09  |

## Ratios:

|                                           |     |
|-------------------------------------------|-----|
| Ni <sup>++</sup> /hypo <sup>-</sup> ..... | 0.4 |
| Tribasic hydroxy-acid/Ni .....            | 0.5 |

Malic acid/Ni<sup>++</sup> .....

|                                   |     |
|-----------------------------------|-----|
| Malic acid/Ni <sup>++</sup> ..... | 1.0 |
|-----------------------------------|-----|

Stabilizing ions: Te<sup>++</sup> .....

|                        |        |   |
|------------------------|--------|---|
| Te <sup>++</sup> ..... | p.p.m. | 1 |
|------------------------|--------|---|

Initial pH adjusted with HCl and NaOH.

Utilizing this bath, properly cleaned steel samples of 60 cm.<sup>2</sup> area were plated. The bath was employed in a continuous plating system having a plating chamber volume of 300 cc., the volume of the bath being 2 liters and the temperature therein being about 99° C.; and the following results were obtained:

|                                    |        |
|------------------------------------|--------|
| 70 Initial pH .....                | 6.80   |
| Final pH .....                     | 6.20   |
| Weight gain .....                  | 1.8397 |
| Rate R $\times 10^4$ .....         | 4.90   |
| Duration of test, min. .....       | 66     |
| 75 Flow rate soln., cc./min. ..... | 60.6   |

In another of these plating tests, an aqueous bath having the particular composition indicated below was employed:

Bath composition:

Bath No. 16—

|                      |        |        |
|----------------------|--------|--------|
| Sodium citrate       | m.p.l. | 0.05   |
| Sodium succinate     | m.p.l. | 0.06   |
| Nickel sulfate       | m.p.l. | 0.0675 |
| Sodium hypophosphite | m.p.l. | 0.225  |

Ratios:

|                                        |      |
|----------------------------------------|------|
| Ni <sup>++</sup> /hypo <sup>-</sup>    | 0.33 |
| Tribasic hydroxy-acid/Ni <sup>++</sup> | 0.74 |

Stabilizing ions:

|                  |        |   |
|------------------|--------|---|
| Pb <sup>++</sup> | p.p.m. | 5 |
| Zn <sup>++</sup> | p.p.m. | 1 |

Initial pH adjusted with NaOH.

Utilizing this bath, properly cleaned steel samples of 60 cm.<sup>2</sup> area were plated. The bath was employed in a continuous plating system having a plating chamber volume of 300 cc., the volume of the bath being 4 liters and the temperature thereof being about 99° C. In this plating test, the plating bath was regenerated after each cycle by the addition of nickel sulfate, sodium hypophosphite and sodium bicarbonate in the reservoir, in the manner disclosed in the Talmey and Crehan patent; and the following results were obtained:

| Cycle No.                 | 1      | 2      | 3      | 4      | 5      | 6      | 7      |
|---------------------------|--------|--------|--------|--------|--------|--------|--------|
| Initial pH                | 7.20   | 7.20   | 7.30   | 7.20   | 6.75   | 6.50   | 6.50   |
| Final pH                  | 6.20   | 6.00   | 6.30   | 6.30   | 6.40   | 6.25   | 6.30   |
| Wt. gain                  | 1.5672 | 1.9073 | 2.3271 | 2.6918 | 1.9498 | 2.1617 | 2.6493 |
| Rate R $\times 10^4$      | 4.70   | 4.74   | 5.40   | 5.10   | 5.00   | 4.14   | 4.33   |
| Duration of cycle (min.)  | 56     | 67     | 72     | 88     | 66     | 87     | 102    |
| Flow rate soln., cc./min. | 71.4   | 60     | 55.5   | 45.5   | 60.6   | 46     | 40     |

In another of these plating tests, an aqueous bath having the particular composition indicated below was employed:

Bath composition:

Bath No. 17—

|                      |        |       |
|----------------------|--------|-------|
| Sodium citrate       | m.p.l. | 0.08  |
| Sodium succinate     | m.p.l. | 0.06  |
| Nickel sulfate       | m.p.l. | 0.09  |
| Sodium hypophosphite | m.p.l. | 0.225 |

Ratios:

|                                        |          |
|----------------------------------------|----------|
| Ni <sup>++</sup> /Hypo <sup>-</sup>    | 0.4      |
| Tribasic hydroxy-acid/Ni <sup>++</sup> | 0.89     |
| Stabilizing ion: Pb <sup>++</sup>      | p.p.m. 5 |

Utilizing this bath, properly cleaned steel samples of 80 cm.<sup>2</sup> area were plated. The bath was employed in a continuous plating system having a plating chamber volume of 300 cc., the volume of the bath being 4 liters and the temperature thereof being about 99° C. In this plating test, the plating bath was regenerated after each cycle by the addition of nickel sulfate, sodium hypophosphite and sodium bicarbonate in the reservoir in the manner

disclosed in the Talmey and Crehan patent; and the following results were obtained:

| Cycle No.                     | 1    | 2    | 3    | 4    |
|-------------------------------|------|------|------|------|
| Initial pH                    | 6.50 | 6.54 | 6.52 | 6.58 |
| Final pH                      | 5.20 | 5.82 | 6.10 | 6.24 |
| Wt. Gain                      | 2.84 | 3.92 | 4.64 | 3.86 |
| Rate, R $\times 10^4$         | 4.32 | 5.56 | 6.17 | 5.80 |
| Duration of cycle (Min.)      | 82   | 88   | 94   | 83   |
| Flow rate soln., cc./min.     | 45   | 42   | 40   | 44   |
| Cumulative Depletion, percent | 12.7 | 30.1 | 50.7 | 67.9 |

This rate of depletion is an arbitrary measure of the amount of nickel taken out, as a deposit, of the original bath.

In another of these plating tests, an aqueous bath having the particular composition indicated below was employed:

Bath composition:

Bath No. 18—

|                      |        |        |
|----------------------|--------|--------|
| Sodium citrate       | m.p.l. | 0.0725 |
| Sodium succinate     | m.p.l. | 0.06   |
| Nickel chloride      | m.p.l. | 0.09   |
| Sodium hypophosphite | m.p.l. | 0.225  |

Ratios:

|                                        |          |
|----------------------------------------|----------|
| Ni <sup>++</sup> /hypo <sup>-</sup>    | 0.4      |
| Tribasic hydroxy-acid/Ni <sup>++</sup> | 0.8      |
| Stabilizing ion: Pb <sup>++</sup>      | p.p.m. 4 |

Utilizing this bath, properly cleaned steel samples of 80 cm.<sup>2</sup> area were plated. The bath was employed in a continuous plating system having a plating chamber volume of 300 cc., the volume of the bath being 6 liters and the temperature thereof being about 99° C. In this plating test the plating bath was regenerated after each cycle by the addition of nickel chloride, sodium hypophosphite and sodium bicarbonate in the reservoir in the manner disclosed in the Talmey and Crehan patent; and the following results were obtained (duplicate tests being reported):

| Cycle No.                 | 1    | 2    | 3    | 4    | 5    |
|---------------------------|------|------|------|------|------|
| Initial pH                | 6.49 | 6.49 | 6.55 | 6.50 | 6.60 |
| Final pH                  | 6.28 | 6.32 | 5.65 | 5.61 | 5.68 |
| Wt. Gain                  | 5.29 | 4.96 | 4.13 | 3.69 | 3.98 |
| Rate, R $\times 10^4$     | 5.60 | 5.25 | 4.45 | 4.39 | 5.08 |
| Duration of Cycle, Min.   | 118  | 118  | 116  | 105  | 98   |
| Flow rate Soln., cc./min. | 49   | 49   | 49   | 54   | 58   |
| Cumul. Depl., Percent     | 16.7 | 14.7 | 28.7 | 26.6 | 41.3 |
|                           |      |      |      | 42.0 | 58.7 |
|                           |      |      |      |      | 56.5 |
|                           |      |      |      |      | 75.6 |
|                           |      |      |      |      | 69.9 |

In another of these plating tests an aqueous bath having the particular composition indicated below was employed:

Bath composition:

Bath No. 19—

|                      |        |       |
|----------------------|--------|-------|
| Sodium citrate       | m.p.l. | 0.045 |
| Sodium aminoacetate  | m.p.l. | 0.09  |
| Nickel chloride      | m.p.l. | 0.09  |
| Sodium hypophosphite | m.p.l. | 0.225 |

Ratios:

|                                        |     |
|----------------------------------------|-----|
| Ni <sup>++</sup> /hypo <sup>-</sup>    | 0.4 |
| Tribasic hydroxy-acid/Ni <sup>++</sup> | 0.5 |

Utilizing this bath, properly cleaned steel samples of 60 cm.<sup>2</sup> area were plated. The bath was employed in a continuous plating system having a plating chamber volume of 300 cc., the volume of the bath being 4 liters and the temperature thereof being about 99° C. In this plating test, the plating bath was regenerated after each cycle by the addition of nickel chloride, sodium hypophosphate and sodium bicarbonate in the reservoir, in the manner disclosed in the Talmey and Crehan patent; and the following results were obtained:

| Cycle No.                     | 1      | 2      |
|-------------------------------|--------|--------|
| Initial pH.....               | 7.00   | 6.80   |
| Final pH.....                 | 6.30   | 6.40   |
| Wt. gain.....                 | 1.2132 | 1.5638 |
| Rate, R $\times 10^4$ .....   | 3.91   | 3.62   |
| Duration of cycle (min.)..... | 52     | 85     |
| Flow rate soln., cc./min..... | 77     | 47.1   |

In another of these plating tests, an aqueous bath having the particular composition indicated below was employed:

Bath composition:

Bath No. 20—

|                            |        |       |    |
|----------------------------|--------|-------|----|
| Sodium citrate .....       | m.p.l. | 0.045 | 25 |
| Sodium aminoacetate .....  | m.p.l. | 0.09  |    |
| Diglycollic acid .....     | m.p.l. | 0.06  |    |
| Nickel chloride .....      | m.p.l. | 0.09  |    |
| Sodium hypophosphate ..... | m.p.l. | 0.225 |    |

Ratios:

|                                        |        |
|----------------------------------------|--------|
| Ni <sup>++</sup> /hypo-                | 0.4    |
| Tribasic hydroxy-acid/Ni <sup>++</sup> | 0.5    |
| Stabilizing ion: Pb <sup>++</sup>      | p.p.m. |

Initial pH adjusted with HCl and NaOH.

Utilizing this bath, properly cleaned steel samples of 60 cm.<sup>2</sup> area were plated. The bath was employed in a continuous plating system having a plating chamber volume of 300 cc., the volume of the bath being 4 liters and the temperature thereof being about 99° C. In this plating test, the plating bath was regenerated after each cycle by the addition of nickel chloride, sodium hypophosphate and sodium bicarbonate in the reservoir, in the manner disclosed in the Talmey and Crehan patent; and the following results were obtained:

| Cycle No.                     | 1      | 2      | 3      | 4     | 5      | 6      | 7      | 8      | 9      |
|-------------------------------|--------|--------|--------|-------|--------|--------|--------|--------|--------|
| Initial pH.....               | 6.80   | 7.20   | 7.18   | 7.20  | 7.15   | 7.50   | 7.15   | 7.40   | 7.50   |
| Final pH.....                 | 6.10   | 6.50   | 6.50   | 6.50  | 6.60   | 7.10   | 6.40   | 6.70   | 6.80   |
| Wt. Gain.....                 | 1.9725 | 1.6111 | 1.9738 | 2.555 | 2.0079 | 2.8350 | 2.9681 | 2.6999 | 2.3011 |
| Rate, R $\times 10^4$ .....   | 4.33   | 4.00   | 5.14   | 5.39  | 5.58   | 5.76   | 6.11   | 6.34   | 6.39   |
| Duration of cycle (min.)..... | 76     | 55     | 64     | 79    | 60     | 82     | 81     | 71     | 60     |
| Flow rate soln., cc./min..... | 52.7   | 72.77  | 62.5   | 50.6  | 66.6   | 48.8   | 49.4   | 56.3   | 66.6   |

Hardness tests were performed upon these samples plated with the Bath No. 20 with results between 600 and 680 Vickers units.

In another of these plating tests, an aqueous bath having the particular composition indicated below was employed:

Bath composition:

Bath No. 21—

|                            |        |       |
|----------------------------|--------|-------|
| Malic acid .....           | m.p.l. | 0.18  |
| Sodium succinate .....     | m.p.l. | 0.06  |
| Nickel sulfate .....       | m.p.l. | 0.09  |
| Sodium hypophosphate ..... | m.p.l. | 0.225 |

Ratios:

|                                        |        |
|----------------------------------------|--------|
| Ni <sup>++</sup> /hypo-                | 0.4    |
| Hydroxy-acid/Ni <sup>++</sup>          | 2.0    |
| Stabilizing ion: Pb <sup>++</sup>      | p.p.m. |
| Initial pH adjusted with HCl and NaOH. | 1.0    |

Utilizing this bath, a properly cleaned steel sample of 20 cm.<sup>2</sup> area was plated for 60 minutes in 100 cc. of the bath at 99° C.; then the bath was regenerated with nickel

75

sulfate and sodium bicarbonate and a new sample of 20 cm.<sup>2</sup> area was plated for 60 minutes in the regenerated bath. The results of these companion tests were as follows:

|                 | Original bath | Regener-<br>ated bath |
|-----------------|---------------|-----------------------|
| Initial pH..... | 5.50          | 5.60                  |
| Final pH.....   | 4.50          | 4.30                  |
| Wt. gain.....   | 0.3215        | 0.3434                |

In another of these plating tests an aqueous bath having the particular composition indicated below was employed:

Bath composition:

Bath No. 22—

|                            |        |       |
|----------------------------|--------|-------|
| Malic acid .....           | m.p.l. | 0.09  |
| Aminoacetic acid .....     | m.p.l. | 0.09  |
| Nickel chloride .....      | m.p.l. | 0.09  |
| Sodium hypophosphate ..... | m.p.l. | 0.225 |

Ratios:

|                               |     |
|-------------------------------|-----|
| Ni <sup>++</sup> /hypo-       | 0.4 |
| Hydroxy-acid/Ni <sup>++</sup> | 1.0 |
| Amino/Ni <sup>++</sup>        | 1.0 |

Stabilizing ions:

|                        |        |     |
|------------------------|--------|-----|
| Pb <sup>++</sup> ..... | p.p.m. | 1.0 |
| Te <sup>++</sup> ..... | p.p.m. | 1.0 |

Initial pH adjusted with NaOH.

Utilizing this bath, properly cleansed steel samples of 60 cm.<sup>2</sup> area were plated. The bath was employed in a continuous plating system having a plating chamber volume of 300 cc., the volume of the bath being 4 liters and the temperature thereof being about 99° C. In this plating test the plating bath was regenerated after each cycle by the addition of nickel chloride, sodium hypophosphate and sodium bicarbonate in the reservoir in the manner disclosed in the Talmey and Crehan patent, and the following results were obtained:

45

Utilizing this bath, properly cleansed steel samples of 60 cm.<sup>2</sup> area were plated. The bath was employed in a continuous plating system having a plating chamber volume of 300 cc., the volume of the bath being 4 liters and the temperature thereof being about 99° C. In this plating test the plating bath was regenerated after each cycle by the addition of nickel chloride, sodium hypophosphate and sodium bicarbonate in the reservoir in the manner disclosed in the Talmey and Crehan patent, and the following results were obtained:

45

| Cycle No.                     | 1      | 2      | 3      | 4      | 5      |
|-------------------------------|--------|--------|--------|--------|--------|
| Initial pH.....               | 6.50   | 6.50   | 7.00   | 6.90   | 6.80   |
| Final pH.....                 | 6.15   | 6.12   | 6.25   | 6.15   | 6.18   |
| Wt. gain.....                 | 0.6837 | 0.8221 | 1.1499 | 2.6252 | 2.6594 |
| Rate R $\times 10^4$ .....    | 4.54   | 4.42   | 4.91   | 4.66   | 4.81   |
| Duration of cycle (min.)..... | 25     | 31     | 39     | 94     | 92     |
| Flow rate Soln., cc./min..... | 80     | 58.1   | 51.3   | 42.6   | 43.7   |

In another of these plating tests an aqueous bath having the particular composition indicated below was employed:

Bath composition:

Bath No. 23—

|                            |        |       |
|----------------------------|--------|-------|
| Malic acid .....           | m.p.l. | 0.18  |
| Sodium succinate .....     | m.p.l. | 0.06  |
| Nickel sulfate .....       | m.p.l. | 0.09  |
| Sodium hypophosphate ..... | m.p.l. | 0.225 |

Ratios:

|                                   |        |
|-----------------------------------|--------|
| Ni <sup>++</sup> /hypo-           | 0.4    |
| Hydroxy-acid/Ni <sup>++</sup>     | 2.0    |
| Stabilizing ion: Pb <sup>++</sup> | p.p.m. |

Initial pH adjusted with HCl and NaOH.

Utilizing this bath, properly prepared general purpose "Bakelite" samples of 70 cm.<sup>2</sup> area were plated. The bath was employed in a continuous plating system having a plating chamber volume of 300 cc., the volume of the bath being 4 liters and the temperature thereof being about 99° C. In this plating test the plating bath was regenerated after each cycle by the addition of nickel

volume of 300 cc., the volume of the bath being 1 liter and the temperature thereof being about 100° C. In this plating test, the plating bath was regenerated after each cycle by the addition of nickel chloride, sodium hypophosphite and sodium bicarbonate in the reservoir in the manner disclosed in the Talmey and Crehan patent; and the following results were obtained:

| Cycle No.                     | 1      | 2      | 3      | 4      | 5      | 6      | 7      | 8      |
|-------------------------------|--------|--------|--------|--------|--------|--------|--------|--------|
| Initial pH                    | 5.40   | 5.38   | 5.39   | 5.37   | 5.33   | 5.37   | 5.38   | 5.44   |
| Final pH                      | 5.00   | 5.08   | 4.91   | 5.07   | 4.99   | 5.11   | 5.07   | 5.28   |
| Wt. gain (gms.)               | 4.69   | 4.11   | 3.62   | 4.82   | 3.56   | 4.03   | 5.00   | 4.96   |
| Time, min.                    | 116    | 105    | 100    | 126    | 94     | 103    | 126    | 121    |
| Soln. flow rate, cc./min.     | 49     | 54     | 57     | 45     | 61     | 55     | 45     | 47     |
| Plating rate, $R \times 10^4$ | 5.04   | 4.90   | 4.53   | 4.77   | 4.18   | 4.90   | 4.96   | 5.13   |
| Turnover of Ni, m.p.l.        | 0.0125 | 0.0235 | 0.0332 | 0.0461 | 0.0556 | 0.0663 | 0.0796 | 0.0929 |

sulfate, sodium hypophosphite and sodium bicarbonate in the reservoir, in the manner disclosed in the Talmey and Crehan patent; and the following results were obtained:

| Cycle No.                 | 1      | 2      | 3      | 4      | 5      | 6      | 7      |
|---------------------------|--------|--------|--------|--------|--------|--------|--------|
| Initial pH                | 5.50   | 5.52   | 5.52   | 5.48   | 5.55   | 5.53   | 5.44   |
| Final pH                  | 5.01   | 5.15   | 5.14   | 5.12   | 5.06   | 5.28   | 5.00   |
| Wt. Gain                  | 4.0370 | 3.6900 | 3.0650 | 3.5880 | 4.3099 | 5.6230 | 4.2290 |
| Rate $R \times 10^4$      |        |        | 3.86   | 4.14   | 4.07   | 4.6    | 4.16   |
| Duration Cycle (min.)     | 150    | 240    | 150    | 240    | 150    | 150    | 140    |
| Flow rate soln., cc./min. | 27     | 22     | 27     | 22     | 27     | 27     | 29     |
| Cumul. Depl. percent      | 19.0   | 36.0   | 50.5   | 67.5   | 87.9   | 106.5  | 135.2  |

Prior to plating the samples of "Bakelite" were prepared in accordance with the methods disclosed in U.S. Patent No. 2,690,401, granted on September 28, 1954, to Gregoire Gutzeit, William J. Crehan and Abraham Krieg, and in U.S. Patent No. 2,690,402, granted on September 28, 1954, to William J. Crehan. Specifically, the outer layer or skins of the "Bakelite" samples were removed mechanically with fine emery cloth; and then they were soaked in an aqueous solution containing 35 p.p.m. of palladium chloride for 72 hours; the samples were then thoroughly rinsed in water, dried, and the palladium chloride was reduced to metallic palladium in a hot aqueous solution of sodium hypophosphite (0.335 m.p.l.) until bubbling subsided. The nickel coatings on the "Bakelite" samples were of excellent quality, bright and smooth, and adhesion was excellent, resisting both thermal shock from -40° C. to 100° C., as well as mechanical shock.

In another of these plating tests an aqueous bath having the particular composition indicated below was employed:

#### Bath composition:

Bath No. 24—

Nickel chloride ..... m.p.l. 0.0675  
Sodium hypophosphite ..... m.p.l. 0.225

In another of these plating tests, an aqueous bath having the particular composition indicated below was employed:

Bath composition:

Bath No. 25—

|                      | M.p.l. |
|----------------------|--------|
| Nickel chloride      | 0.0675 |
| Sodium hypophosphite | 0.225  |
| Malic acid           | 0.06   |
| Lactic acid          | 0.2025 |
| Sodium succinate     | 0.12   |
| Phosphorous acid     | 0.4    |

No lead added for stabilization, because lactic acid (and commercial  $NiCl_2$ ) contain sufficient lead as impurity (0.7 p.p.m. in bath).

Utilizing this bath, properly cleaned steel samples of 80 cm.<sup>2</sup> area are plated. The bath was employed in a continuous plating system having a plating chamber volume of 300 cc., the volume of the bath being 9 liters and the temperature thereof being about 100° C. In this plating test, the plating bath was regenerated after each cycle by the addition of nickel chloride, sodium hypophosphite and sodium bicarbonate in the reservoir, in the manner disclosed in the Talmey and Crehan patent; and initially 0.4 m.p.l. of phosphite ions were introduced into the bath for the purpose of examining the ability of the bath to hold phosphite at a reasonably high phosphite ion concentration.

The results of this test were as follows:

| Cycle No.                      | 1    | 2    | 3    | 4    | 5    | 6    | 7    |
|--------------------------------|------|------|------|------|------|------|------|
| Initial pH                     | 4.74 | 4.74 | 4.72 | 4.75 | 4.75 | 4.73 | 4.77 |
| Final pH                       | 4.59 | 4.69 | 4.62 | 4.61 | 4.60 | 4.66 | 4.68 |
| Wt. gain, gms.                 | 4.67 | 3.68 | 4.00 | 3.80 | 3.75 | 4.07 | 4.20 |
| Time, min.                     | 120  | 101  | 95   | 88   | 105  | 123  | 127  |
| Soln. Flow rate, cc./min.      | 47   | 56   | 60   | 65   | 64   | 46   | 46   |
| Plating rate, $R \times 10^4$  | 4.85 | 4.55 | 5.08 | 5.40 | 4.45 | 4.14 | 4.14 |
| Addition of $Pb^{++}$ , p.p.m. | None | None | None | 1    | None | None | None |

Malic acid ..... m.p.l. 0.135  
Sodium succinate ..... m.p.l. 0.06  
 $Pb^{++}$  as stabilizing ion ..... p.p.m. 2.0  
(Water to make one liter of solution.)

In passing, it is noted that the plating rate which was up to  $4.5 \times 10^{-4}$  gm./cm.<sup>2</sup>/min. in cycle No. 4 dropped to  $4.14 \times 10^{-4}$  gm./cm.<sup>2</sup>/min. in cycle No. 5, after the feeding into the bath of only 1 p.p.m. of  $Pb^{++}$ . Even as little as 0.25 p.p.m. of  $Pb^{++}$  may result in a drop of the plating rate from about  $5.0 \times 10^{-4}$  to  $4.5 \times 10^{-4}$  gm./cm.<sup>2</sup>/min. in Bath No. 25. On the other hand, the Bath No. 25 does not respond disadvantageously, as to

Utilizing this bath properly cleaned steel samples of 80 cm.<sup>2</sup> area were plated. The bath was employed in a continuous plating system having a plating chamber

plating rate, to the addition of other stabilizing ions and molecules (Te<sup>++</sup> etc., sulfhydric compounds, etc.) as disclosed in the copending application of Paul Talmey and Gregoire Gutzeit, Serial No. 359,428, filed June 3, 1953.

In another series of these plating tests, an aqueous bath having the particular composition indicated below was employed:

Bath composition:

Bath No. 26—

|                                         |        |        |
|-----------------------------------------|--------|--------|
| Nickel (as chloride) .....              | m.p.l. | 0.0675 |
| Sodium hypophosphite .....              | m.p.l. | 0.225  |
| Glycerol .....                          | m.p.l. | 0.135  |
| Stabilizing ion: Pb <sup>++</sup> ..... | p.p.m. | 1      |
| pH adjusted with NaOH or HCl.           |        |        |

It is noted that two molecules of glycerol can complex three molecules of nickel; whereby the polyalcohol in the Bath No. 26 is in excess.

Utilizing this plating bath, properly cleaned steel samples of 20 cm.<sup>2</sup> area were plated for 10 minutes and 60 minutes, the volume of the bath being 50 cc. and the temperature thereof being about 99° C., with the following results:

| Plating time.....                   | 10 minutes      |               |                                     | 60 minutes      |               |                                     |
|-------------------------------------|-----------------|---------------|-------------------------------------|-----------------|---------------|-------------------------------------|
|                                     | Initial pH..... | Wt. gain..... | Plating rate, R $\times 10^4$ ..... | Initial pH..... | Wt. gain..... | Plating rate, R $\times 10^4$ ..... |
| Initial pH.....                     | 4.50            | 5.00          | 5.50                                | 4.50            | 5.00          | 5.50                                |
| Wt. gain.....                       | 0.0095          | 0.01          | 0.016                               | 0.0274          | 0.0345        | 0.0434                              |
| Plating rate, R $\times 10^4$ ..... | 0.48            | 0.50          | 0.80                                | none            | none          | none                                |
| Turbidity.....                      | none            | none          | none                                | none            | none          | none                                |

In view of the foregoing, it will be understood that the bath containing glycerol alone, in amounts sufficient to complex completely the nickel ions, gives 10 minute plating rates below  $1.0 \times 10^{-4}$  gm./cm.<sup>2</sup>/min.

A plating bath (No. 27), identical to the Bath No. 26 (except that it also contained 0.06 m.p.l. of sodium succinate) was then prepared; and utilizing this plating bath properly cleaned steel samples of 20 cm.<sup>2</sup> area were plated for 10 minutes and 60 minutes, the volume of the bath being 50 cc. and the temperature thereof being about 99° C., with the following results:

| Plating time.....                   | 10 minutes      |               |                                     | 60 minutes      |               |                                     |
|-------------------------------------|-----------------|---------------|-------------------------------------|-----------------|---------------|-------------------------------------|
|                                     | Initial pH..... | Wt. gain..... | Plating rate, R $\times 10^4$ ..... | Initial pH..... | Wt. gain..... | Plating rate, R $\times 10^4$ ..... |
| Initial pH.....                     | 4.50            | 5.0           | 4.50                                | 4.50            | 5.0           | 5.0                                 |
| Wt. gain.....                       | 0.0673          | 0.0995        | 0.1216                              | 0.1216          | 0.1590        | 0.1590                              |
| Plating rate, R $\times 10^4$ ..... | 3.36            | 4.98          | none                                | none            | none          | none                                |
| Turbidity.....                      | none            | none          | none                                | none            | none          | none                                |

In another series of these plating tests, an aqueous bath having the particular composition indicated below was employed:

Bath composition:

Bath No. 28—

|                               | M.p.l. |
|-------------------------------|--------|
| Nickel chloride .....         | 0.0675 |
| Sodium hypophosphite .....    | 0.225  |
| Mannitol .....                | 0.135  |
| pH adjusted with NaOH or HCl. |        |

Utilizing this bath, properly cleaned steel samples of 20 cm.<sup>2</sup> area were plated for 10 minutes and 60 minutes, the volume of the bath being 50 cc. and the temperature thereof being about 99° C., with the following results:

| Plating time.....                   | 10 minutes      |               |                                     | 60 minutes      |               |                                     |
|-------------------------------------|-----------------|---------------|-------------------------------------|-----------------|---------------|-------------------------------------|
|                                     | Initial pH..... | Wt. gain..... | Plating rate, R $\times 10^4$ ..... | Initial pH..... | Wt. gain..... | Plating rate, R $\times 10^4$ ..... |
| Initial pH.....                     | 4.5             | 5.0           | 5.5                                 | 4.5             | 5.0           | 5.5                                 |
| Wt. gain.....                       | 0.0088          | 0.0088        | 0.015                               | 0.0304          | 0.0350        | 0.0441                              |
| Plating rate, R $\times 10^4$ ..... | 0.44            | 0.44          | 0.75                                | none            | none          | none                                |
| Turbidity.....                      | none            | none          | none                                | none            | none          | none                                |

In view of the foregoing, it will be understood that the plating bath containing mannitol alone, in amounts

sufficient to complex completely the nickel ions, gives 10 minute plating rates below  $1.0 \times 10^{-4}$  gm./cm.<sup>2</sup>/min.

A plating bath (No. 29), identical to the Bath No. 28 (except that it also contained 0.06 m.p.l. of sodium succinate and 1.0 p.p.m. of Pb<sup>++</sup> as stabilizing ion) was then prepared; and utilizing this plating bath properly cleaned steel samples of 20 cm.<sup>2</sup> area were plated for 10 minutes and 60 minutes, the volume of the bath being 50 cc. and the temperature thereof being about 99° C., with the following results:

| Plating time.....                   | 10 minutes      |               | 60 minutes      |               |
|-------------------------------------|-----------------|---------------|-----------------|---------------|
|                                     | Initial pH..... | Wt. gain..... | Initial pH..... | Wt. gain..... |
| Initial pH.....                     | 4.50            | 5.0           | 4.50            | 5.0           |
| Wt. gain.....                       | 0.0716          | 0.0890        | 0.1215          | 0.1598        |
| Plating rate, R $\times 10^4$ ..... | 3.58            | 4.45          | none            | none          |
| Turbidity.....                      | none            | none          | none            | none          |

In another series of these plating tests, an aqueous bath having the particular composition indicated below was employed:

Bath composition:

Bath No. 30—

|                                         |        |        |
|-----------------------------------------|--------|--------|
| Nickel chloride .....                   | m.p.l. | 0.0675 |
| Sodium hypophosphite .....              | m.p.l. | 0.225  |
| Pyruvic acid .....                      | m.p.l. | 0.135  |
| Sodium succinate .....                  | m.p.l. | 0.06   |
| Stabilizing ion: Pb <sup>++</sup> ..... | p.p.m. | 1.0    |
| pH adjusted with NaOH and HCl.          |        |        |

Utilizing this plating bath, properly cleaned steel samples of 20 cm.<sup>2</sup> area were plated for 10 minutes and 60 minutes, the volume of the bath being 50 cc. and the temperature thereof being about 99° C., with the following results:

| Plating time.....                   | 10 minutes      |               | 60 minutes      |               |
|-------------------------------------|-----------------|---------------|-----------------|---------------|
|                                     | Initial pH..... | Wt. gain..... | Initial pH..... | Wt. gain..... |
| Initial pH.....                     | 4.48            | 4.97          | 4.48            | 4.97          |
| Wt. gain.....                       | 0.0702          | 0.0694        | 0.1572          | 0.1686        |
| Plating rate, R $\times 10^4$ ..... | 3.47            | 3.51          | none            | none          |
| Turbidity.....                      | none            | none          | none            | none          |

In these plating tests, it will be observed that the 10 minute rates are relatively low, however, the weight of plating deposited in one hour is quite high. This indicated a long initiation period for the plating reaction.

In another series of these plating tests, an aqueous bath having the particular composition indicated below was employed:

Bath composition:

Bath No. 31—

|                                         |        |        |
|-----------------------------------------|--------|--------|
| Nickel chloride .....                   | m.p.l. | 0.0675 |
| Sodium hypophosphite .....              | m.p.l. | 0.225  |
| Levulinic acid .....                    | m.p.l. | 0.2025 |
| Sodium succinate .....                  | m.p.l. | 0.06   |
| Stabilizing ion: Pb <sup>++</sup> ..... | p.p.m. | 1.0    |
| pH adjusted with NaOH.                  |        |        |

It is noted that the amount of levulinic acid is more than that needed to complex all of the nickel ions in the plating bath (about 50% excess).

Utilizing this bath, properly cleaned steel samples of 20 cm.<sup>2</sup> area were plated for 10 minutes and 60 minutes, the volume of the bath being 50 cc. and the temperature thereof being about 99° C., with the following results:

| Plating time.....                   | 10 minutes      |               |                                     | 60 minutes      |               |                                     |
|-------------------------------------|-----------------|---------------|-------------------------------------|-----------------|---------------|-------------------------------------|
|                                     | Initial pH..... | Wt. gain..... | Plating rate, R $\times 10^4$ ..... | Initial pH..... | Wt. gain..... | Plating rate, R $\times 10^4$ ..... |
| Initial pH.....                     | 4.00            | 4.52          | 5.02                                | 4.00            | 4.52          | 5.02                                |
| Wt. gain.....                       | 0.0667          | 0.0968        | 0.0872                              | 0.1422          | 0.1870        | 0.2065                              |
| Plating rate, R $\times 10^4$ ..... | 3.34            | 4.84          | 4.36                                | none            | none          | none                                |
| Turbidity.....                      | none            | none          | none                                | none            | none          | none                                |

In passing, it is noted that very high weights of plating are deposited in one hour at pH 4.50 and 5.0.

In another series of these plating tests, an aqueous bath having the particular composition indicated below was employed:

Bath composition:

Bath No. 32—

Nickel chloride ..... m.p.l. 0.0675  
 Sodium hypophosphite ..... m.p.l. 0.225  
 Trimethylamine ..... m.p.l. 0.135  
 Stabilizing ion: Pb<sup>++</sup> ..... p.p.m. 1.0  
 pH adjusted with HCl.

To the Bath No. 32 increasing amounts of sodium succinate were added from 0 to 0.09 m.p.l. and corresponding plating tests were performed on properly cleaned steel samples of 20 cm.<sup>2</sup> areas for 10 minutes and 60 minutes, the volume of the bath being 50 cc. and the temperature thereof being about 99° C., with the following results:

15 20

In view of the foregoing, it will be observed that the optimum pH for the Bath No. 33 appears to be around

|                               |        |        |        |        |
|-------------------------------|--------|--------|--------|--------|
| Succinate, m.p.l.             | none   |        | 0.03   |        |
| Plating time (min.)           | 10     | 60     | 10     | 60     |
| Initial pH                    | 4.66   | 4.60   | 4.52   | 4.52   |
| Weight gain                   | 0.0044 | 0.0344 | 0.0588 | 0.1052 |
| Plating rate, R $\times 10^4$ | 0.22   | 2.94   | none   | none   |
| Turbidity                     | none   | none   | none   | none   |
| Succinate, m.p.l.             | .06    |        | .09    |        |
| Plating time (min.)           | 10     | 60     | 10     | 60     |
| Initial pH                    | 3.93   | 4.5    | 5.04   | 3.93   |
| Weight gain                   | 0.0610 | 0.0841 | 0.0926 | 0.1104 |
| Plating rate, R $\times 10^4$ | 3.05   | 4.20   | 4.63   | none   |
| Turbidity                     | none   | none   | none   | none   |

In view of the foregoing, it will be observed that the chelating of the nickel ions in the Bath No. 32 gives exceedingly low plating rates, which are boosted by the addition of the proper amount of the exaltant at the proper pH.

In another series of these plating tests, an aqueous bath having the particular composition indicated below was employed:

Bath composition:

Bath No. 33—

Nickel chloride ..... m.p.l. 0.0675  
 Sodium hypophosphite ..... m.p.l. 0.225  
 Propylenediamine ..... m.p.l. 0.0675  
 Stabilizing ion: Pb<sup>++</sup> ..... p.p.m. 1.0  
 pH adjusted with HCl.

To the Bath No. 33 increasing amounts of sodium succinate were added from 0 to 0.09 m.p.l. and corresponding plating tests were performed on properly cleaned steel samples of 20 cm.<sup>2</sup> area for 10 minutes and 60 minutes, the volume of the bath being 50 cc. and the temperature thereof being about 99° C., with the following results:

45

5.0 and that the addition of succinate over about 0.06 m.p.l does not appear to give an equivalent improvement.

In another of these plating tests, an aqueous bath having the particular composition indicated below was employed:

Bath composition:

Bath No. 34—

Nickel chloride ..... m.p.l. 0.0675  
 Sodium hypophosphite ..... m.p.l. 0.225  
 Sodium succinate ..... m.p.l. 0.06  
 Propylenediamine ..... m.p.l. 0.0675  
 Stabilizing ion: Pb<sup>++</sup> ..... p.p.m. 1.0  
 pH adjusted with HCl.

50 55

Utilizing this plating bath, properly cleaned steel samples of 80 cm.<sup>2</sup> area were plated, the bath was employed in a continuous plating system having a plating chamber volume of 300 cc., the volume of the bath being 4 liters and the temperature thereof being 98° C.-99° C. The pH of the bath was 5.0 and the test was conducted for 120 minutes; the weight gain was 3.9941 gms.; and the plating was smooth and bright with good adhesion. In this plating test, the calculated plating rate was 4.16 $\times 10^{-4}$  gm./cm.<sup>2</sup>/min.

In another series of these plating tests, an aqueous bath having the particular composition indicated below was employed:

Bath composition:

Bath No. 35—

Nickel chloride ..... m.p.l. 0.0675  
 Sodium hypophosphite ..... m.p.l. 0.225  
 1-2 aminoethanol ..... m.p.l. 0.135  
 Stabilizing ion: Pb<sup>++</sup> ..... p.p.m. 1.0  
 pH adjusted with HCl.

70 75

|                               |        |        |        |        |
|-------------------------------|--------|--------|--------|--------|
| Succinate, m.p.l.             | None   |        | 0.03   |        |
| Plating time (min.)           | 10     | 60     | 10     | 60     |
| Initial pH                    | 5.03   | 5.03   | 5.03   | 5.03   |
| Wt. gain                      | 0.0185 | 0.0472 | 0.0694 | 0.1242 |
| Plating rate, R $\times 10^4$ | 0.92   | 3.47   | none   | none   |
| Turbidity                     | none   | none   | none   | none   |

To the Bath No. 35 increasing amounts of sodium succinate were added from 0 to 0.09 m.p.l. and corresponding plating tests were performed on properly cleaned steel samples of 20 cm.<sup>2</sup> area for 10 minutes, the volume of the bath being 50 cc. and the temperature thereof being about 99° C., with the following results:

| Sodium Succinate m.p.l.         | None   |        |        | 0.03   |        |
|---------------------------------|--------|--------|--------|--------|--------|
| Initial pH                      | 3.50   | 4.00   | 4.50   | 3.52   | 4.05   |
| Wt. gain                        | 0.0078 | 0.0108 | 0.01   | 0.0140 | 0.0326 |
| Plating rate, R×10 <sup>4</sup> | 0.39   | 0.54   | 0.50   | 0.70   | 1.63   |
| Turbidity                       | none   | none   | none   | none   | 2.18   |
| Sodium Succinate, m.p.l.        | 0.06   |        |        |        |        |
| Initial pH                      | 3.48   | 4.05   | 4.52   | 4.95   |        |
| Wt. gain                        | 0.0128 | 0.0408 | 0.0562 | 0.1067 |        |
| Plating rate, R×10 <sup>4</sup> | 0.64   | 2.04   | 2.81   | 5.34   |        |
| Turbidity                       | none   | none   | none   | none   |        |
| Sodium Succinate m.p.l.         | 0.09   |        |        |        |        |
| Initial pH                      | 3.53   | 4.03   | 4.45   | 5.02   |        |
| Wt. gain                        | 0.0247 | 0.0523 | 0.0760 | 0.0881 |        |
| Plating rate, R×10 <sup>4</sup> | 1.24   | 2.62   | 3.80   | 4.46   |        |
| Turbidity                       | none   | none   | none   | none   |        |

Substantially identical plating tests were performed using the Bath No. 35 during 60 minutes with the following results:

| Sodium Succinate, m.p.l. | 0.06   | 0.09   |        |        |
|--------------------------|--------|--------|--------|--------|
| Initial pH               | 4.95   | 3.53   | 4.03   | 4.45   |
| Wt. gain                 | 0.2024 | 0.0247 | 0.0523 | 0.0760 |

In the Bath No. 35, it was observed that the pH appears to be rather critical in that the plating rates of  $2.81 \times 10^{-4}$  and  $5.34 \times 10^{-4}$  gm./cm.<sup>2</sup>/min. correspond to the pH values of 4.52 and 4.95 at a level of 0.06 m.p.l. of succinate.

In another series of these plating tests, an aqueous bath having the particular composition indicated below was employed:

Bath composition:

Bath No. 36—

|                                   |        |        |
|-----------------------------------|--------|--------|
| Nickel chloride                   | m.p.l. | 0.0675 |
| Sodium hypophosphite              | m.p.l. | 0.225  |
| Sodium succinate                  | m.p.l. | 0.06   |
| Morpholine                        | m.p.l. | 0.135  |
| Stabilizing ion: Pb <sup>++</sup> | p.p.m. | 1.0    |
| pH adjusted with HCl.             |        |        |

Utilizing this plating bath, properly cleaned steel samples of 20 cm.<sup>2</sup> area were plated for 10 minutes and 60 minutes, the volume of the bath being 50 cc. and the temperature thereof being about 99° C., with the following results:

| Time of plating (min.)          | 10     | 60     | 10     | 60     |
|---------------------------------|--------|--------|--------|--------|
| Initial pH                      | 4.50   | 4.50   | 5.00   | 5.00   |
| Wt. gain                        | 0.0594 | 0.1208 | 0.770  | 0.1488 |
| Plating rate, R×10 <sup>4</sup> | 2.97   | none   | 3.85   | none   |
| Turbidity                       | none   | none   | none   | none   |
| Time of Plating (min.)          | 10     | 60     | 10     | 60     |
| Initial pH                      | 5.50   | 5.50   | 5.95   | 5.95   |
| Wt. gain                        | 0.0921 | 0.1752 | 0.0925 | 0.1874 |
| Plating rate, R×10 <sup>4</sup> | 4.60   | none   | 4.62   | none   |
| Turbidity                       | none   | none   | none   | none   |

In another series of these plating tests, an aqueous bath having the particular composition indicated below was employed:

Bath composition:

Bath No. 37—

|                 |        |        |
|-----------------|--------|--------|
| Nickel chloride | m.p.l. | 0.0675 |
|-----------------|--------|--------|

|                                   |        |        |
|-----------------------------------|--------|--------|
| Sodium hypophosphite              | m.p.l. | 0.225  |
| Semi-carbazide                    | m.p.l. | 0.0675 |
| Stabilizing ion: Pb <sup>++</sup> | p.p.m. | 1.0    |
| pH adjusted with HCl.             |        |        |

To the Bath No. 37 increasing amounts of sodium succinate were added from 0 to 0.09 m.p.l. and corresponding plating tests were performed on properly cleaned steel samples of 20 cm.<sup>2</sup> area were plated for 10 minutes and 60 minutes, the volume of the bath being 50 cc. and the temperature thereof being about 99° C., with the following results:

| Succinate, m.p.l.               | none   |        | 0.03   |        |
|---------------------------------|--------|--------|--------|--------|
| Plating time (min.)             | 10     | 60     | 10     | 60     |
| Initial pH                      | 5.04   | 5.04   | 5.00   | 5.00   |
| Wt. gain                        | 0.0035 | 0.0166 | 0.0636 | 0.0969 |
| Plating rate, R×10 <sup>4</sup> | 0.18   | 3.18   | 3.61   | none   |
| Turbidity                       | none   | none   | none   |        |
| Succinate, m.p.l.               | 0.06   |        |        |        |
| Plating time (min.)             | 10     | 60     | 10     | 60     |
| Initial pH                      | 4.53   | 4.53   | 5.00   | 5.00   |
| Wt. gain                        | 0.0624 | 0.1150 | 0.0722 | 0.1396 |
| Plating rate, R×10 <sup>4</sup> | 3.12   | none   | 3.61   | none   |
| Turbidity                       | none   | none   | none   |        |
| Succinate, m.p.l.               | 0.09   |        |        |        |
| Plating time (min.)             | 10     | 60     | 10     | 60     |
| Initial pH                      | 5.50   | 5.50   | 5.03   | 5.03   |
| Wt. gain                        | 0.0720 | 0.1549 | 0.074  | 0.1644 |
| Plating rate, R×10 <sup>4</sup> | 3.60   | none   | 3.70   | none   |
| Turbidity                       | none   | none   | none   |        |

It is noted that in the Bath No. 37 with 0.06 m.p.l. of succinate and at a pH of 5.5, the 10 minute rate is substantially equal to that obtained at a pH of 5.0, but that in the 60 minute plating tests the weight gain of the plating is substantially higher at the higher pH.

In another series of these plating tests, an aqueous bath having the particular composition indicated below was employed:

Bath composition:

Bath No. 38—

|                                   |        |        |
|-----------------------------------|--------|--------|
| Nickel chloride                   | m.p.l. | 0.0675 |
| Sodium hypophosphite              | m.p.l. | 0.225  |
| Sodium succinate                  | m.p.l. | 0.06   |
| Aminoacetic acid (glycine)        | m.p.l. | 0.135  |
| Stabilizing ion: Pb <sup>++</sup> | p.p.m. | 1.0    |
| pH adjusted with HCl and NaOH.    |        |        |

Utilizing this plating bath, properly cleaned steel samples of 20 cm.<sup>2</sup> area were plated for 10 minutes and 60 minutes, the volume of the bath being 50 cc. and the temperature thereof being about 99° C., with the following results:

| Initial pH                     | 4.50   |        | 5.00   |        | 5.62   |        |
|--------------------------------|--------|--------|--------|--------|--------|--------|
| Plating time (min.)            | 10     | 60     | 10     | 60     | 10     | 60     |
| Initial pH                     | 5.50   | 5.50   | 5.95   | 5.95   |        |        |
| Wt. gain                       | 0.0833 | 0.1810 | 0.0940 | 0.1956 | 0.0924 | 0.2104 |
| Plating rate R×10 <sup>4</sup> | 4.17   | -----  | 4.70   | -----  | 4.67   | -----  |
| Initial pH                     | 6.05   |        | 6.52   |        | 7.02   |        |
| Plating time (min.)            | 10     | 60     | 10     | 60     | 10     | 60     |
| Initial pH                     | 6.05   | 6.52   | 7.02   |        |        |        |
| Wt. gain                       | 0.0946 | 0.2080 | 0.0985 | 0.2043 | 0.0912 | 0.2021 |
| Plating rate R×10 <sup>4</sup> | 4.73   | -----  | 4.79   | -----  | 4.56   | -----  |

In another series of these plating tests, an aqueous bath having the particular composition indicated below was employed:

## Bath composition:

## Bath No. 39—

|                            |        |        |
|----------------------------|--------|--------|
| Nickel chloride            | m.p.l. | 0.0675 |
| Sodium hypophosphite       | m.p.l. | 0.225  |
| Sodium succinate           | m.p.l. | 0.06   |
| Beta-alanine               | m.p.l. | 0.135  |
| Stabilizing ion: $Pb^{++}$ | p.p.m. | 1.0    |

pH adjusted with NaOH and HCl.

Utilizing this plating bath, properly cleaned steel samples of 20 cm.<sup>2</sup> area were plated for 10 minutes and 60 minutes, the volume of the bath being 50 cc. and the temperature thereof being about 99° C., with the following results:

|                               |        |        |        |        |        |        |
|-------------------------------|--------|--------|--------|--------|--------|--------|
| Initial pH                    | 4.50   |        | 5.05   |        | 5.52   |        |
| Plating time (min.)           | 10     | 60     | 10     | 60     | 10     | 60     |
| Wt. gain                      | 0.0772 | 0.1508 | 0.0052 | 0.1854 | 0.0966 | 0.1991 |
| Plating rate, $R \times 10^4$ |        | 3.86   | 4.76   | 4.63   |        |        |
| Initial pH                    | 6.03   |        | 6.45   |        |        |        |
| Plating time (min.)           | 10     | 60     | 10     | 60     |        |        |
| Wt. gain                      | 0.0942 | 0.1985 | 0.0922 | 0.1993 |        |        |
| Plating rate, $R \times 10^4$ | 4.71   | 4.61   |        |        |        |        |

In another of these plating tests, an aqueous bath having the particular composition indicated below was employed:

## Bath composition:

## Bath No. 40—

|                            |        |       |
|----------------------------|--------|-------|
| Nickel chloride            | m.p.l. | 0.09  |
| Sodium hypophosphite       | m.p.l. | 0.225 |
| Malic acid                 | m.p.l. | 0.09  |
| Aminoacetic acid           | m.p.l. | 0.09  |
| Stabilizing ion: $Pb^{++}$ | p.p.m. | 2     |

Utilizing this plating bath properly cleaned steel samples of 80 cm.<sup>2</sup> area were plated. The bath was employed in a continuous plating system having a plating chamber volume of 300 cc., the volume of the bath being 1 liter and the temperature thereof being about 100° C. In this plating test, the plating bath was regenerated after each cycle by the addition of nickel chloride, sodium hypophosphite and sodium hydroxide in the reservoir, in the manner disclosed in the Talmey and Crehan patent, and the following results were obtained:

| Cycle No.                     | 1    | 2    | 3    | 4    |
|-------------------------------|------|------|------|------|
| Initial pH                    | 6.80 | 6.80 | 6.78 | 6.80 |
| Final pH                      | 6.08 | 5.98 | 6.26 | 6.21 |
| Wt. gain, gms.                | 3.81 | 4.65 | 3.68 | 3.80 |
| Time, min.                    | 94   | 114  | 92   | 100  |
| Soln. flow rate, cc./min.     | 61   | 50   | 62   | 56   |
| Plating rate, $R \times 10^4$ | 5.06 | 6.10 | 5.00 | 4.75 |

35 After the sixth and twelfth cycles 0.009 m.p.l. of aminoacetic acid were added (10%).

Also it is noted that the plating rate of the Bath No. 40 is dependent upon the phosphite concentration, whereby the plating rate actually improves as the continuous operation proceeds without resulting in nickel phosphite precipitation.

In another of these plating tests, an aqueous bath having the particular composition indicated below was employed:

45 Bath composition:

Bath No. 41—

|                      |        |        |
|----------------------|--------|--------|
| Nickel chloride      | m.p.l. | 0.0675 |
| Sodium hypophosphite | m.p.l. | 0.225  |
| Malic acid           | m.p.l. | 0.135  |
| Aminoacetic acid     | m.p.l. | 0.0675 |
| Stabilizing ion:     |        |        |
| $Pb^{++}$            | p.p.m. | 2.0    |
| $Te^{++}$            | p.p.m. | 1.0    |

50 Utilizing this plating bath properly cleaned steel samples of 80 cm.<sup>2</sup> area were plated. The bath was employed in a continuous plating system having a plating chamber volume of 300 cc., the volume of the bath being 1 liter and the temperature thereof being about 100° C. In this plating test, the plating bath was regenerated after each cycle by the addition of nickel chloride, sodium hypophosphite and sodium hydroxide in the reservoir, in the manner disclosed in the Talmey and Crehan patent, and the following results were obtained:

| Cycle No.                     | 1      | 2      | 3      | 4      | 5      | 6      | 7    |
|-------------------------------|--------|--------|--------|--------|--------|--------|------|
| Initial pH                    | 6.50   | 6.45   | 6.68   | 6.51   | 6.45   | 6.22   | 5.98 |
| Final pH                      | 5.60   | 5.80   | 5.99   | 5.99   | 5.69   | 5.90   | 5.82 |
| Wt. gain, gms.                | 4.76   | 5.36   | 5.41   | 6.28   | 7.64   | 6.14   | 4.50 |
| Time, min.                    | 120    | 100    | 96     | 100    | 123    | 110    | 100  |
| Soln. flow rate, cc./min.     | 47     | 57     | 59     | 57     | 46     | 52     | 57   |
| Plating rate, $R \times 10^4$ | 4.97   | 6.70   | 7.02   | 7.84   | 7.75   | 16.96  | 5.63 |
| Turnover, m.p.l.              | 0.0127 | 0.0270 | 0.0414 | 0.0590 | 0.0808 | 0.0972 |      |

<sup>1</sup> Addition of 2.0 p.p.m.  $Pb^{++}$  and 1.0 p.p.m.  $Te^{++}$ .

| Cycle No.                     | 5    | 6    | 7    | 8    | 9    |
|-------------------------------|------|------|------|------|------|
| Initial pH                    | 6.81 | 6.50 | 6.50 | 6.50 | 6.50 |
| Final pH                      | 6.31 | 6.20 | 6.20 | 6.20 | 6.20 |
| Wt. gain, gms.                | 3.94 | 1.95 | 2.38 | 2.37 | 2.31 |
| Time, min.                    | 102  | 65   | 73   | 74   | 74   |
| Soln. flow rate, cc./min.     | 50   | 61.5 | 55   | 54   | 55   |
| Plating rate, $R \times 10^4$ | 4.83 | 5.00 | 5.42 | 5.32 | 5.28 |

| Cycle No.                     | 10   | 11   | 12   | 13   |
|-------------------------------|------|------|------|------|
| Initial pH                    | 6.55 | 6.55 | 6.30 | 6.50 |
| Final pH                      | 6.17 | 6.30 | 6.00 | 6.30 |
| Wt. gain, gms.                | 2.59 | 2.86 | 3.61 | 3.03 |
| Time, min.                    | 78   | 77   | 99   | 81   |
| Soln. flow rate, cc./min.     | 51.3 | 52   | 40   | 50   |
| Plating rate, $R \times 10^4$ | 5.53 | 6.19 | 6.09 | 6.23 |

| Cycle No.                     | 14    | 15   | 16   | 17   | 18   |
|-------------------------------|-------|------|------|------|------|
| Initial pH                    | 6.70  | 6.50 | 6.51 | 6.49 | 6.28 |
| Final pH                      | 6.50  | 5.80 | 6.27 | 6.11 | 6.07 |
| Wt. gain, gms.                | 1.20  | 2.71 | 3.09 | 3.39 | 4.18 |
| Time, min.                    | 82    | 71   | 71   | 74   | 86   |
| Soln. flow rate, cc./min.     | 49    | 52   | 52   | 60   | 43   |
| Plating rate, $R \times 10^4$ | 12.45 | 4.75 | 5.43 | 5.72 | 5.93 |

<sup>1</sup> Excess of stabilizing ions (10.0 p.p.m.).

| Cycle No.                    | 19   | 20   | 21   | 22   | 23   |
|------------------------------|------|------|------|------|------|
| Initial pH                   | 6.27 | 5.99 | 6.00 | 6.48 | 6.50 |
| Final pH                     | 6.01 | 5.80 | 5.80 | 6.20 | 6.18 |
| Wt. gain, gms.               | 4.04 | 4.86 | 4.49 | 6.01 | 5.31 |
| Time, min.                   | 77   | 88   | 75   | 90   | 85   |
| Soln. flow rate, cc./min.    | 48   | 42   | 49   | 49   | 44   |
| Plating rate $R \times 10^4$ | 6.55 | 6.93 | 7.35 | 8.33 | 7.83 |

55 After the sixth and twelfth cycles 0.009 m.p.l. of aminoacetic acid were added (10%).

Also it is noted that the plating rate of the Bath No. 40 is dependent upon the phosphite concentration, whereby the plating rate actually improves as the continuous operation proceeds without resulting in nickel phosphite precipitation.

In another of these plating tests, an aqueous bath having the particular composition indicated below was employed:

Bath composition:

Bath No. 41—

Nickel chloride m.p.l. 0.0675

Sodium hypophosphite m.p.l. 0.225

Malic acid m.p.l. 0.135

Aminoacetic acid m.p.l. 0.0675

Stabilizing ion:

$Pb^{++}$  p.p.m. 2.0

$Te^{++}$  p.p.m. 1.0

For the purpose of establishing a standard of comparison, a simple aqueous citric acid plating bath of the present type was prepared that had the following composition:

## Bath composition:

## Bath No. 42—

|                      | M.p.l. |
|----------------------|--------|
| Nickel chloride      | 0.0675 |
| Sodium hypophosphite | 0.225  |
| Citric acid          | 0.0675 |

In a number of portions of Bath No. 42 at different pH, adjusted with NaOH and HCl, each having a volume of

5

## Bath composition:

## Bath No. 43—

| M.p.l. |
|--------|
| 0.0675 |
| 0.225  |
| 0.135  |

10

In a number of portions of Bath No. 43 at different pH, adjusted with NaOH and HCl, each having a volume of 50 cc. and a temperature of about 100° C., properly cleaned steel samples, each of a total area of 20 cm.<sup>2</sup>, were plated in 10 minute rate tests with the following results:

| Initial pH                    | 5.08           | 5.53           | 5.91           | 6.55           | 7.02           |
|-------------------------------|----------------|----------------|----------------|----------------|----------------|
| Wt. gain (g.)                 | 0.0580         | 0.0622         | 0.0632         | 0.0700         | 0.0648         |
| Plating rate, R $\times 10^4$ | 2.90           | 3.11           | 3.16           | 3.50           | 3.24           |
| Plating time (min.)           | 10             | 10             | 10             | 10             | 10             |
| Final pH                      | 4.31           | 4.41           | 4.43           | 4.42           | 4.50           |
| Bath appear. (hot)            | clear, green.  | clear, green.  | clear, green.  | turbid, green. | green.         |
| Bath appear. (cold)           | do             | do             | do             | do             | do             |
| Black precip.                 | none           | none           | none           | none           | none           |
| Plating appear                | smooth, bright | smooth, bright | smooth, bright | smooth, bright | smooth, bright |

50 cc. and at a temperature of about 100° C., properly cleaned steel samples, each of a total area of 20 cm.<sup>2</sup>, were plated in 10 minute rate tests with the following results:

| Initial pH                    | 4.98           | 5.49           | 6.02           | 6.53           | 7.03           | 8.60           |
|-------------------------------|----------------|----------------|----------------|----------------|----------------|----------------|
| Wt. gain (g.)                 | 0.0260         | 0.0311         | 0.0347         | 0.0400         | 0.0401         | 0.0750         |
| Plating rate, R $\times 10^4$ | 1.30           | 1.56           | 1.74           | 2.00           | 2.00           | 3.75           |
| Plating time (Min.)           | 10             | 10             | 10             | 10             | 10             | 10             |
| Final pH                      | 4.18           | 4.20           | 4.20           | 4.21           | 4.40           | 5.60           |
| Bath appear. (hot)            | clear, green.  | clear, green.  | clear, green.  | clear, green.  | clear, green.  | Do.            |
| Bath appear. (cold)           | do             | do             | do             | do             | do             | yes.           |
| Black precip.                 | none           | none           | none           | none           | none           | none           |
| Plating appear                | smooth, bright | smooth, bright | smooth, bright | smooth, bright | smooth, bright | smooth, bright |

The simple aqueous citric acid Bath No. 42 was modified by adding thereto different exaltants, each in the amount of 0.0675 m.p.l. and similar 10 minute plating rate tests were conducted on identical properly cleaned steel samples with the following results:

rate tests were conducted on identical properly cleaned steel samples with the following results:

| Exaltant                      | Glycine        | Alpha-alanine  | Alpha-amino-butyric acid | Aspartic acid  |
|-------------------------------|----------------|----------------|--------------------------|----------------|
| Wt. gain (g.)                 | 0.0594         | 0.0880         | 0.0402                   | 0.0461         |
| Plating rate, R $\times 10^4$ | 2.97           | 4.40           | 2.01                     | 2.31           |
| Plating time (min.)           | 10             | 10             | 10                       | 10             |
| Initial pH                    | 6.48           | 7.07           | 5.42                     | 6.82           |
| Final pH                      | 5.42           | 5.95           | 4.47                     | 5.72           |
| Bath appear. (hot)            | clear, blue.   | clear, blue.   | green.                   | blue.          |
| Bath appear. (cold)           | do             | do             | do                       | do             |
| Black precip.                 | none           | none           | none                     | none           |
| Plating appear                | smooth, bright | smooth, bright | smooth, bright           | smooth, bright |

45

50

55

60

65

75

| Exaltant                      | Glycine        | Alpha-alanine  | Alpha-amino-butyric acid | Aspartic acid  |
|-------------------------------|----------------|----------------|--------------------------|----------------|
| Wt. gain (g.)                 | 0.0846         | 0.0729         | 0.0646                   | 0.0641         |
| Plating rate, R $\times 10^4$ | 4.23           | 3.65           | 3.23                     | 3.31           |
| Plating time (min.)           | 10             | 10             | 10                       | 10             |
| Initial pH                    | 6.42           | 6.08           | 5.42                     | 6.96           |
| Final pH                      | 4.92           | 4.78           | 4.58                     | 5.43           |
| Bath appear. (hot)            | clear, blue.   | clear, blue.   | clear, green.            | clear, blue.   |
| Bath appear. (cold)           | do             | do             | do                       | do             |
| Black precip.                 | none           | none           | none                     | none           |
| Plating appear                | smooth, bright | smooth, bright | smooth, bright           | smooth, bright |

  

| Exaltant                      | Malonic acid   | Succinic acid  | Glutaric acid  | Adipic acid    |
|-------------------------------|----------------|----------------|----------------|----------------|
| Wt. gain (g.)                 | 0.0732         | 0.0723         | 0.0638         | 0.0615         |
| Plating rate, R $\times 10^4$ | 3.66           | 3.62           | 3.28           | 3.08           |
| Plating time (min.)           | 10             | 10             | 10             | 10             |
| Initial pH                    | 5.52           | 5.05           | 5.62           | 4.86           |
| Final pH                      | 4.88           | 4.63           | 4.76           | 3.08           |
| Bath appear. (hot)            | clear, green.  | clear, green.  | clear, green.  | clear, green.  |
| Bath appear. (cold)           | do             | do             | do             | do             |
| Black precip.                 | none           | none           | none           | none           |
| Plating appear                | smooth, bright | smooth, bright | smooth, bright | smooth, bright |

For the purpose of demonstrating the exalting effects of a number of simple short chain saturated aliphatic monocarboxylic acids, further plating tests were conducted involving a number of plating baths of the nickel cation-hypophosphite anion type containing various ones of the chelating agents previously described; and in these tests in each instance a volume of 50 cc. of the bath

For the purpose of establishing a standard of comparison a simple aqueous malic acid plating bath of the present type was prepared that had the following composition:

was employed at a temperature of about 100° C., and properly cleaned steel samples were used, each having a total area of 20 cm.<sup>2</sup>, and each of the tests being conducted for a time interval of ten minutes.

In a first series of these plating tests, an aqueous plating bath was employed that had the following composition:

| Bath No. 44:         | M.p.l. |
|----------------------|--------|
| Nickel sulfate       | 0.08   |
| Sodium hypophosphite | 0.23   |
| Hydroxyacetic acid   | 0.20   |

In these plating tests, Bath No. 44 was used containing no propionic acid (as a standard) and different quantities of propionic acid as indicated below and with the following results:

| Propionic acid (m.p.l.)       | none   | 0.03   | 0.06   |
|-------------------------------|--------|--------|--------|
| Initial pH                    | 4.6    | 4.6    | 4.6    |
| Weight gain (g.)              | 0.0589 | 0.0649 | 0.0752 |
| Plating rate, R $\times 10^4$ | 2.95   | 3.25   | 3.76   |
| Final pH                      | 4.0    | 4.0    | 4.0    |

In a second series of these plating tests, an aqueous plating bath was employed that had the following composition:

| Bath No. 45:         | M.p.l. |
|----------------------|--------|
| Nickel sulfate       | 0.08   |
| Sodium hypophosphite | 0.23   |
| Malic acid           | 0.16   |

In these plating tests, Bath No. 45 was used containing no propionic acid (as a standard) and different quantities of propionic acid as indicated below and with the following results:

| Propionic acid (m.p.l.)       | none   | 0.03   | 0.06   |
|-------------------------------|--------|--------|--------|
| Initial pH                    | 4.62   | 4.63   | 4.60   |
| Weight gain (g.)              | 0.0591 | 0.0617 | 0.0664 |
| Plating rate, R $\times 10^4$ | 2.95   | 3.08   | 3.32   |
| Final pH                      | 4.1    | 4.4    | 4.5    |

In a third series of these plating tests, an aqueous plating bath was employed that had the following composition:

| Bath No. 46:         | M.p.l. |
|----------------------|--------|
| Nickel sulfate       | 0.08   |
| Sodium hypophosphite | 0.23   |
| Lactic acid          | 0.20   |

In these plating tests, Bath No. 46 was used containing no propionic acid (as a standard) and different quantities of propionic acid as indicated below and with the following results:

| Propionic acid (m.p.l.)       | none   | 0.03   | 0.06   |
|-------------------------------|--------|--------|--------|
| Initial pH                    | 4.63   | 4.60   | 4.60   |
| Weight gain (g.)              | 0.0584 | 0.0783 | 0.0843 |
| Plating rate, R $\times 10^4$ | 3.42   | 3.91   | 4.21   |
| Final pH                      | 4.0    | 3.9    | 4.0    |

In a fourth series of these plating tests, an aqueous plating bath was employed that had the following composition:

| Bath No. 47:         | M.p.l. |
|----------------------|--------|
| Nickel sulfate       | 0.08   |
| Sodium hypophosphite | 0.23   |
| Aminoacetic acid     | 0.16   |

In these plating tests, Bath No. 47 was used containing no propionic acid (as a standard) and different quantities of propionic acid as indicated below with the following results:

| Propionic acid (m.p.l.)       | none   | 0.03   | 0.06   |
|-------------------------------|--------|--------|--------|
| Initial pH                    | 6.20   | 6.22   | 6.20   |
| Weight gain (g.)              | 0.0812 | 0.0972 | 0.1040 |
| Plating rate, R $\times 10^4$ | 4.06   | 4.86   | 5.20   |
| Final pH                      | 5.5    | 5.5    | 5.4    |

In a fifth series of these plating tests, an aqueous plating bath was employed that had the following composition:

| Bath No. 48:         | M.p.l. |
|----------------------|--------|
| Nickel sulfate       | 0.08   |
| Sodium hypophosphite | 0.23   |
| Propylenediamine     | 0.16   |

In these plating tests, Bath No. 48 was used containing no propionic acid (as a standard) and different quantities of propionic acid as indicated below and with the following results:

| Propionic acid (m.p.l.)       | none   | 0.03   | 0.06   |
|-------------------------------|--------|--------|--------|
| Initial pH                    | 4.64   | 4.65   | 4.64   |
| Weight gain (g.)              | 0.0175 | 0.0300 | 0.0370 |
| Plating rate, R $\times 10^4$ | 0.88   | 1.50   | 1.85   |
| Final pH                      | 3.4    | 4.1    | 4.2    |

In additional series of these plating tests, Bath No. 46 was again employed containing different amounts of butyric acid and valeric acid as indicated below and with the following results:

| Butyric acid (m.p.l.)         | 0.03   | 0.06   | 0.03   | 0.06   |
|-------------------------------|--------|--------|--------|--------|
| Valeric acid (m.p.l.)         | 4.64   | 4.62   | 4.64   | 4.60   |
| Initial pH                    | 0.0740 | 0.0803 | 0.0749 | 0.0856 |
| Weight gain (g.)              | 3.70   | 4.01   | 3.75   | 4.28   |
| Plating rate, R $\times 10^4$ | 4.0    | 4.0    | 4.0    | 4.0    |

In a further series of these plating tests, Bath No. 47 was again employed containing different amounts of butyric acid and valeric acid as indicated below and with the following results:

| Butyric acid (m.p.l.)         | 0.03   | 0.06   | 0.03   | 0.06   |
|-------------------------------|--------|--------|--------|--------|
| Valeric acid (m.p.l.)         | 6.24   | 6.22   | 6.20   | 6.20   |
| Initial pH                    | 0.0921 | 0.0996 | 0.0902 | 0.0936 |
| Weight gain (g.)              | 4.61   | 4.98   | 4.51   | 4.48   |
| Plating rate, R $\times 10^4$ | 5.4    | 5.5    | 5.4    | 5.4    |

In each of these series of plating tests involving as exalting additives the various simple short chain saturated aliphatic monocarboxylic acids, the nickel platings produced were smooth and bright and excellent in character.

Summarizing these data it may be derived that the functional relationship between the plating rate and the concentration of organic acid used as an exalting additive in the plating bath is expressed by the linear equation:

$$(1) \log R = mc_a + R_0$$

where:

$R$  = plating rate

$c_a$  = concentration of organic acid

$m$  = slope

$R_0$  = intercept constant or unexalted plating rate.

Differentiation of (1) yields the equation:

$$(2) \frac{1}{R} \frac{dR}{dc_a} = m$$

The value of  $m$  is a definite functional property of the organic acid used as an exalting additive, and the numerical value thereof indicates the degree of exaltation of the normal or unexalted plating rate of the particular plating bath by the particular organic acid.

Recapitulating, in the continuous plating system, the malic acid-lactic acid-succinate bath, the malic acid-glycine bath and the malic acid-succinate bath are generally preferred both from the standpoint of economy and performance. Specifically, the malic acid-lactic acid-succinate plating bath, although somewhat slower than the other two last-mentioned plating baths with regard to plating rate, is productive of a nickel plating upon steel that exhibits excellent adhesion (even on steel castings) as it may be employed at a pH as low as 4.0 to

5.0, and since this plating bath has a long useful life, as it will retain nickel phosphite in solution even at concentrations up to 1 molar. Specifically, the malic acid-glycine plating bath exhibits an exceedingly high plating rate and retains the nickel phosphite in solution over the exceedingly wide pH range 4.3 to 9.5 even in a concentration as high as 1 molar. Specifically, the malic acid-succinate bath has an entirely satisfactory plating rate and an optimum pH substantially at neutrality and satisfactorily holds the nickel phosphite in solution even at a concentration as high as 1 molar.

A typical malic acid-lactic acid-succinate plating bath comprises: an absolute concentration of hypophosphite ions in the range 0.15 to 1.20 moles/liter; a ratio between nickel ions and hypophosphite ions in the range 0.25 to 1.60; an absolute concentration of malic acid ions in the range 0.04 to 0.20 mole/liter; an absolute concentration of lactic acid ions in the range 0.04 to 0.20 mole/liter; the total quantity of the malic acid ions and the lactic acid ions are sufficient to complex at least 100% of the nickel ions; an absolute concentration of succinic acid ions of at least 0.04 mole/liter; and a pH within the range 4.0 to 7.0.

A typical malic acid-glycine plating bath comprises: an absolute concentration of hypophosphite ions in the range 0.15 to 1.20 mole/liter; a ratio between nickel ions and the hypophosphite ions in the range 0.25 to 1.60; an absolute concentration of malic acid ions sufficient to complex at least 100% of the nickel ions; an absolute concentration of glycine ions of at least 0.04 mole/liter; and a pH within the range 4.3 to 9.5.

A typical malic acid-succinate plating bath comprises: an absolute concentration of hypophosphite ions in the range 0.15 to 1.20 mole/liter; a ratio between nickel ions and hypophosphite ions in the range 0.25 to 1.60; an absolute concentration of malic acid ions sufficient to complex at least 100% of the nickel ions; an absolute concentration of succinic acid ions of at least 0.04 mole/liter; and a pH within the range 4.0 to 7.0.

In view of the foregoing, it is apparent that there has been provided an improved process of chemical nickel plating, as well as improved plating baths therefor, wherein the baths are of the nickel cation-hypophosphite anion type, also containing a chelating agent of the character specified and substantially completely chelating all of the nickel ions in the bath, and also containing an exalting additive of the character specified and exalting the plating rate of the bath. The chelating agent is selected from the group having the general formula:



where: R is an aliphatic radical, X is a functional group containing a dissociable hydrogen atom and selected from the class consisting of:



and Y is a functional group containing a negative atom acting as a center of coordination and selected from the class consisting of:



and wherein the functional groups X and Y are in alpha or beta positions to each other. The exalting additive is selected from the group consisting of simple short chain saturated aliphatic monocarboxylic acids including 3 to 5 carbon atoms and salts thereof, simple short chain saturated aliphatic dicarboxylic acids including 3 to 6 carbon atoms and salts thereof, and short chain aliphatic amino carboxylic acids and salts thereof. The plating baths are particularly well-adapted for use in a continuous plating system as they exhibit a fast plating rate, have an exceedingly long life, and maintain nickel phosphite in solution in concentrations as high as one molar.

While there has been described what is at present considered to be the preferred embodiment of the invention, it will be understood that various modifications may be made therein, and it is intended to cover in the appended claims all such modifications as fall within the true spirit and scope of the invention.

What is claimed is:

1. The process of chemically plating with nickel a body comprising an element selected from the group consisting of iron, cobalt, nickel, aluminum, copper, silver, gold, palladium and platinum, which comprises contacting said body with a bath comprising an aqueous solution of a nickel salt and a hypophosphite and a first chelating agent selected from the group consisting of malic acid and salts thereof and a second chelating agent selected from the group consisting of lactic acid and salts thereof and an exalting additive selected from the group consisting of succinic acid and salts thereof, the ratio between nickel ions and hypophosphite ions in said bath being in the range 0.25 to 1.60, the absolute concentration of hypophosphite ions in said bath being in the range 0.15 to 1.20 mole/liter, the absolute concentration of malic acid ions in said bath being in the range 0.04 to 0.20 mole/liter, the absolute concentration of lactic acid ions in said bath being in the range 0.04 to 0.20 mole/liter, the total quantity of said first and second chelating agents in said bath being sufficient to chelate at least 100% of the nickel ions therein so as to impart to said bath a phosphite tolerance of at least about 1 mole/liter, and the absolute concentration of succinic acid ions in said bath being at least 0.04 mole/liter so as substantially to exalt the plating rate of said bath.

2. The process of chemically plating with nickel a body comprising an element selected from the group consisting of iron, cobalt, nickel, aluminum, copper, silver, gold, palladium and platinum, which comprises contacting said body with a hot bath comprising a aqueous solution of a nickel salt and a hypophosphite and a first chelating agent selected from the group consisting of malic acid and salts thereof and a second chelating agent selected from the group consisting of lactic acid and salts thereof and an exalting additive selected from the group consisting of succinic acid and salts thereof, the temperature of said bath being above 90° C. and the pH of said bath being in the range 4.0 to 7.0, the ratio between nickel ions and hypophosphite ions in said bath being in the range 0.25 to 1.60 the absolute concentration of hypophosphite ions in said bath being in the range 0.15 to 1.20 moles/liter, the absolute concentration of malic acid ions in said bath being in the range 0.04 to 0.20 mole/liter, the absolute concentration of lactic acid ions in said bath being in the range 0.04 to 0.20 mole/liter, the total quantity of said first and second chelating agents in said bath being sufficient to chelate at least 100% of the nickel ions therein so as to impart to said bath a phosphite tolerance of at least about 1 mol/liter, and the absolute concentration of succinic acid ions in said bath being at least 0.04 mol/liter so as substantially to exalt the plating rate of said bath.

3. The process of chemically plating with nickel a body essentially comprising an element selected from the group consisting of iron, cobalt, nickel, aluminum, copper, silver, gold, palladium and platinum, which comprises contacting said body with a bath comprising an aqueous solution of nickel ions, hypophosphite ions, a chelating agent, and a separate and different chemical type exalting additive; said agent being present in an amount sufficient to chelate at least 100% of the nickel ions in said bath so as to impart thereto a phosphite tolerance of at least about 1 mole/liter and having the general formula:



- 75 where: R is an aliphatic radical, X is a functional group

containing a dissociable hydrogen atom and selected from the class consisting of:



and Y is a functional group containing a negative atom acting as a center of coordination and selected from the class consisting of:



and wherein the functional groups X and Y are in alpha or beta positions to each other; said additive being present in an amount sufficient substantially to exalt the plating rate of said bath and being selected from the group consisting of simple short chain saturated aliphatic monocarboxylic acids including 3 to 5 carbon atoms and salts thereof, simple short chain saturated aliphatic dicarboxylic acids including 3 to 6 carbon atoms and salts thereof, and short chain aliphatic aminocarboxylic acids and salts thereof; wherein the absolute concentration of hypophosphite ions in said bath expressed in mole/liter is within the range 0.15 to 1.20, the ratio between nickel ions and hypophosphite ions in said bath expressed in molar concentrations is within the range 0.25 to 1.60 and the initial pH of said bath is within the approximate range 4.0 to 11.0.

4. The process of chemically plating with nickel a body essentially comprising an element selected from the group consisting of iron, cobalt, nickel, aluminum, copper, silver, gold, palladium and platinum, which comprises contacting said body with a bath comprising an aqueous solution of a nickel salt, an alkaline hypophosphite, a chelating agent, and a separate and different chemical type exalting additive; said agent being present in an amount sufficient to chelate at least 100% of the nickel ions in said bath so as to impart thereto a phosphite tolerance of at least about 1 mole/liter and having the general formula:



where: R is an aliphatic radical, X is a functional group containing a dissociable hydrogen atom and selected from the class consisting of:



and Y is a functional group containing a negative atom acting as a center of coordination and selected from the class consisting of:



and wherein the functional groups X and Y are in alpha or beta positions to each other; said additive being present in an amount sufficient substantially to exalt the plating rate of said bath and being selected from the group consisting of simple short chain saturated aliphatic monocarboxylic acids including 3 to 5 carbon atoms and salts thereof, simple short chain saturated aliphatic dicarboxylic acids including 3 to 6 carbon atoms and salts thereof, and short chain aliphatic aminocarboxylic acids and salts thereof; wherein the absolute concentration of hypophosphite ions in said bath expressed in mole/liter is within the range 0.15 to 1.20, the ratio between nickel ions and hypophosphite ions in said bath expressed in molar concentrations is within the range of 0.25 to 1.60, and the initial pH of said bath is within the approximate range 4.0 to 11.0.

5. The process of chemically plating with nickel a body essentially comprising an element selected from the group consisting of iron, cobalt, nickel, aluminum, copper, silver, gold, palladium and platinum, which comprises contacting said body with a bath comprising an aqueous solution of nickel ions, hypophosphite ions, a chelating agent, and a separate and different chemical type exalting additive; said agent being present in an

amount sufficient to chelate at least 100% of the nickel ions in said bath so as to impart thereto a phosphite tolerance of at least about 1 mole/liter and having the general formula:



where: R is an aliphatic radical, X is a functional group containing a dissociable hydrogen atom and selected from the class consisting of:



and Y is a functional group containing a negative atom acting as a center of coordination and selected from the class consisting of:



and wherein the functional groups X and Y are in alpha or beta positions to each other; said additive being present in an amount sufficient substantially to exalt the plating rate of said bath and being selected from the group consisting of simple short chain saturated aliphatic monocarboxylic acids including 3 to 5 carbon atoms and salts

thereof, simple short chain saturated aliphatic dicarboxylic acids including 3 to 6 carbon atoms and salts thereof, and short chain aliphatic aminocarboxylic acids and salts thereof; wherein the absolute concentration of hypophosphite ions in said bath expressed in mole/liter is within the range 0.15 to 1.20, the ratio between nickel ions and hypophosphite ions in said bath expressed in molar concentrations is within the range 0.25 to 1.60, and the initial pH of said bath is within the approximate range 4.0 to 11.0

6. The process of chemically plating with nickel a body essentially comprising an element selected from the group consisting of iron, cobalt, nickel, aluminum, copper, silver, gold, palladium and platinum, which comprises contacting said body with a bath comprising an aqueous solution of nickel ions, hypophosphite ions, a chelating agent, and a separate and different chemical type exalting additive; said agent being present in an amount sufficient to chelate at least 100% of the nickel ions in said bath so as to impart thereto a phosphite

tolerance of at least about 1 mole/liter and being selected from the group consisting of saturated aliphatic hydroxycarboxylic acids and salts thereof; said additive being present in an amount sufficient substantially to exalt the plating rate of said bath and being selected from the group consisting of simple short chain saturated aliphatic monocarboxylic acids including 3 to 5 carbon atoms and salts thereof, simple short chain saturated aliphatic dicarboxylic acids including 3 to 6 carbon atoms and salts thereof, and short chain aliphatic aminocarboxylic acids and salts thereof; wherein the absolute concentration of hypophosphite ions in said bath expressed in mole/liter is within the range 0.15 to 1.20, the ratio between nickel ions and hypophosphite ions in said bath expressed in molar concentrations is within the range 0.25 to 1.60, and the initial pH of said bath is within the approximate range 4.0 to 7.0

7. The process of chemically plating with nickel a body essentially comprising an element selected from the group consisting of iron, cobalt, nickel, aluminum, copper, silver, gold, palladium and platinum, which comprises contacting said body with a bath comprising an aqueous solution of nickel ions, hypophosphite ions, a chelating agent, and a separate and different chemical type exalting additive; said agent being present in an amount sufficient to chelate at least 100% of the nickel ions in said bath so as to impart thereto a phosphite tolerance of at least about 1 mole/liter and being selected from the group consisting of saturated aliphatic hydroxycarboxylic acids and salts thereof; said additive being present in an amount sufficient substantially to exalt the

75

plating rate of said bath and being selected from the group consisting of simple short chain saturated aliphatic monocarboxylic acids including 3 to 5 carbon atoms and salts thereof; wherein the absolute concentration of hypophosphite ions in said bath expressed in mole/liter is within the range 0.15 to 1.20, the ratio between nickel ions and hypophosphite ions in said bath expressed in molar concentrations is within the range 0.25 to 1.60, and the initial pH of said bath is within the approximate range 4.0 to 7.0.

8. The process of chemically plating with nickel a body essentially comprising an element selected from the group consisting of iron, cobalt, nickel, aluminum, copper, silver, gold, palladium and platinum, which comprises contacting said body with a bath comprising an aqueous solution of nickel ions, hypophosphite ions, a chelating agent, and a separate and different chemical type exalting additive; said agent being present in an amount sufficient to chelate at least 100% of the nickel ions in said bath so as to impart thereto a phosphite tolerance of at least about 1 mole/liter and being selected from the group consisting of saturated aliphatic hydroxycarboxylic acids and salts thereof; said additive being present in an amount sufficient substantially to exalt the plating rate of said bath and being selected from the group consisting of simple short chain saturated aliphatic dicarboxylic acids including 3 to 6 carbon atoms and salts thereof; wherein the absolute concentration of hypophosphite ions in said bath expressed in mole/liter is within the range 0.15 to 1.20, the ratio between nickel ions and hypophosphite ions in said bath expressed in molar concentrations is within the range 0.25 to 1.60, and the initial pH of said bath is within the approximate range 4.0 to 7.0.

9. The process of chemically plating with nickel a body essentially comprising an element selected from the group consisting of iron, cobalt, nickel, aluminum, copper, silver, gold, palladium and platinum, which comprises contacting said body with a bath comprising an aqueous solution of nickel ions, hypophosphite ions, a chelating agent, and a separate and different chemical type exalting additive; said agent being present in an amount sufficient to chelate at least 100% of the nickel ions in said bath so as to impart thereto a phosphite tolerance of at least about 1 mole/liter and being selected from the group consisting of lactic acid and salts thereof; said additive being present in an amount sufficient substantially to exalt the plating rate of said bath and being selected from the group consisting of succinic acid and salts thereof; wherein the absolute concentration of hypophosphite ions in said bath expressed in mole/liter is within the range 0.15 to 1.20, the ratio between nickel ions and hypophosphite ions in said bath expressed in molar concentrations is within the range 0.25 to 1.60, and the initial pH of said bath is within the approximate range 4.0 to 7.0.

10. The process of chemically plating with nickel a body essentially comprising an element selected from the group consisting of iron, cobalt, nickel, aluminum, copper, silver, gold, palladium and platinum, which comprises contacting said body with a bath comprising an aqueous solution of nickel ions, hypophosphite ions, a chelating agent, and a separate and different chemical type exalting additive; said agent being present in an amount sufficient to chelate at least 100% of the nickel ions in said bath so as to impart thereto a phosphite tolerance of at least about 1 mole/liter and being selected from the group consisting of malic acid and salts thereof; said additive being present in an amount sufficient substantially to exalt the plating rate of said bath and being selected from the group consisting of succinic acid and salts thereof; wherein the absolute concentration of hypophosphite ions in said bath expressed in mole/liter is within the range 0.15 to 1.20, the ratio between nickel ions and hypophosphite ions in said bath expressed in molar concentrations is within the range 0.25 to 1.60, and the initial pH of said bath is within the approximate range 4.0 to 7.0.

range 0.25 to 1.60, and the initial pH of said bath is within the approximate range 4.0 to 7.0.

11. The process of chemically plating with nickel a body essentially comprising an element selected from the group consisting of iron, cobalt, nickel, aluminum, copper, silver, gold, palladium and platinum, which comprises contacting said body with a bath comprising an aqueous solution of a nickel salt and a hypophosphite and a chelating agent selected from the group consisting of malic acid and salts thereof and an exalting additive selected from the group consisting of succinic acid and salts thereof, the ratio between nickel ions and hypophosphite ions in said bath being in the range 0.25 to 1.60, the absolute concentration of hypophosphite ions in said bath being in the range 0.15 to 1.20 mole/liter, the absolute concentration of malic acid ions in said bath being sufficient to chelate at least 100% of the nickel ions therein so as to impart to said bath a phosphite tolerance of at least about 1 mole/liter, and the absolute concentration of succinic acid ions in said bath being at least 0.04 mole/liter so as substantially to exalt the plating rate of said bath.

12. The process of chemically plating with nickel a body comprising an element selected from the group consisting of iron, cobalt, nickel, aluminum, copper, silver, gold, palladium and platinum, which comprises contacting said body with a hot bath comprising an aqueous solution of a nickel salt and a hypophosphite and a chelating agent selected from the group consisting of malic acid and salts thereof and an exalting additive selected from the group consisting of succinic acid and salts thereof, the temperature of said bath being above 90° C. and the pH of said bath being in the range 4.0 to 7.0, the ratio between nickel ions and hypophosphite ions in said bath being in the range 0.25 to 1.60, the absolute concentration of hypophosphite ions in said bath being in the range 0.15 to 1.20 mole/liter, the absolute concentration of malic acid ions in said bath being sufficient to chelate at least 100% of the nickel ions therein so as to impart to said bath a phosphite tolerance of at least about 1 mole/liter, and the absolute concentration of succinic acid ions in said bath being at least 0.04 mole/liter so as substantially to exalt the plating rate of said bath.

13. The process of chemically plating with nickel a body essentially comprising an element selected from the group consisting of iron, cobalt, nickel, aluminum, copper, silver, gold, palladium and platinum, which comprises contacting said body with a bath comprising an aqueous solution of nickel ions, hypophosphite ions, a chelating agent, and a separate and different chemical type exalting additive; said agent being present in an amount sufficient to chelate at least 100% of the nickel ions in said bath so as to impart thereto a phosphite tolerance of at least about 1 mole/liter and being selected from the group consisting of saturated aliphatic hydroxycarboxylic acids and salts thereof; said additive being present in an amount sufficient substantially to exalt the plating rate of said bath and being selected from the group consisting of short chain aliphatic aminocarboxylic acids and salts thereof; wherein the absolute concentration of hypophosphite ions in said bath expressed in mole/liter is within the range 0.15 to 1.20, the ratio between nickel ions and hypophosphite ions in said bath expressed in molar concentrations is within the range 0.25 to 1.60, and the initial pH of said bath is within the approximate range 4.3 to 9.5.

14. The process of chemically plating with nickel a body essentially comprising an element selected from the group consisting of iron, cobalt, nickel, aluminum, copper, silver, gold, palladium and platinum, which comprises contacting said body with a bath comprising an aqueous solution of nickel ions, hypophosphite ions, a chelating agent, and a separate and different chemical type exalting additive; said agent being present in an amount sufficient to chelate at least 100% of the nickel ions in said bath

so as to impart thereto a phosphite tolerance of at least about 1 mole/liter and being selected from the group consisting of malic acid and salts thereof; said additive being present in an amount sufficient substantially to exalt the plating rate of said bath and being selected from the group consisting of aminoacetic acid and salts thereof; wherein the absolute concentration of hypophosphite ions in said bath expressed in mole/liter is within the range 0.15 to 1.20, the ratio between nickel ions and hypophosphite ions in said bath expressed in molar concentrations is within the range 0.25 to 1.60, and the initial pH of said bath is within the approximate range 4.3 to 9.5.

15. The process of chemically plating with nickel a body essentially comprising an element selected from the group consisting of iron, cobalt, nickel, aluminum, copper, silver, gold, palladium and platinum, which comprises contacting said body with a bath comprising an aqueous solution of a nickel salt and a hypophosphite and a chelating agent selected from the group consisting of malic acid and salts thereof and an exalting additive selected from the group consisting of glycine and salts thereof, the ratio between nickel ions and hypophosphite ions in said bath being in the range 0.25 to 1.60, the absolute concentration of hypophosphite ions in said bath being in the range 0.15 to 1.20 moles/liter, the absolute concentration of malic acid ions in said bath being sufficient to chelate at least 100% of the nickel ions therein so as to impart to said bath a phosphite tolerance of at least about 1 mole/liter, and the absolute concentration of glycine ions in said bath being at least 0.04 mole/liter so as substantially to exalt the plating rate of said bath.

16. The process of chemically plating with nickel a body essentially comprising an element selected from the group consisting of iron, cobalt, nickel, aluminum, copper, silver, gold, palladium and platinum, which comprises contacting said body with a hot bath comprising an aqueous solution of a nickel salt and a hypophosphite and a chelating agent selected from the group consisting of malic acid and salts thereof and an exalting additive selected from the group consisting of glycine and salts thereof, the temperature of said bath being above 90° C. and the pH of said bath being in the range 4.3 to 9.5, the ratio between nickel ions and hypophosphite ions in said bath being in the range 0.25 to 1.60, the absolute concentration of hypophosphite ions in said bath being in the range 0.15 to 1.20 moles/liter, the absolute concentration of malic acid ions in said bath being sufficient to chelate at least 100% of the nickel ions therein so as to impart to said bath a phosphite tolerance of at least about 1 mole/liter, and the absolute concentration of glycine ions in said bath being at least 0.04 mole/liter so as substantially to exalt the plating rate of said bath.

17. The process of chemically plating with nickel a body essentially comprising an element selected from the group consisting of iron, cobalt, nickel, aluminum, copper, silver, gold, palladium and platinum, which comprises contacting said body with a bath comprising an aqueous solution of nickel ions, hypophosphite ions, a chelating agent, and a separate and different chemical type exalting additive; said agent being present in an amount sufficient to chelate at least 100% of the nickel ions in said bath so as to impart thereto a phosphite tolerance of at least about 1 mole/liter and being selected from the group consisting of simple short chain aliphatic aminocarboxylic acids and salts thereof; said additive being present in an amount sufficient substantially to exalt the plating rate of said bath and being selected from the group consisting of simple short chain saturated aliphatic monocarboxylic acids including 3 to 5 carbon atoms and salts thereof, and simple short chain saturated aliphatic dicarboxylic acids including 3 to 6 carbon atoms and salts thereof; wherein the absolute concentration of hypophosphite ions in said bath expressed in mole/liter is within the range 0.15 to 1.20, the ratio between nickel ions and hypophosphite ions in said bath expressed in molar concentrations is within the

range 0.25 to 1.60, and the initial pH of said bath is within the approximate range 4.0 to 7.0.

18. The process of chemically plating with nickel a body essentially comprising an element selected from the group consisting of iron, cobalt, nickel, aluminum, copper, silver, gold, palladium and platinum, which comprises contacting said body with a bath comprising an aqueous solution of nickel ions, hypophosphite ions, a chelating agent, and a separate and different chemical type exalting additive; said agent being present in an amount sufficient to chelate at least 100% of the nickel ions in said bath so as to impart thereto a phosphite tolerance of at least about 1 mole/liter and being selected from the group consisting of simple short chain aliphatic aminocarboxylic acids and salts thereof, said additive being present in an amount sufficient substantially to exalt the plating rate of said bath and being selected from the group consisting of simple short chain saturated aliphatic dicarboxylic acids including 3 to 6 carbon atoms and salts thereof; wherein the absolute concentration of hypophosphite ions in said bath expressed in mole/liter is within the range 0.15 to 1.20, the ratio between nickel ions and hypophosphite ions in said bath expressed in molar concentrations is within the range 0.25 to 1.60, and the initial pH of said bath is within the approximate range 4.0 to 7.0.

19. The process of chemically plating with nickel a body essentially comprising an element selected from the group consisting of iron, cobalt, nickel, aluminum, copper, silver, gold, palladium and platinum, which comprises contacting said body with a bath comprising an aqueous solution of nickel ions, hypophosphite ions, a chelating agent, and a separate and different chemical type exalting additive; said agent being present in an amount sufficient to chelate at least 100% of the nickel ions in said bath so as to impart thereto a phosphite tolerance of at least about 1 mole/liter and being selected from the group consisting of aminoacetic acid and salts thereof; said additive being present in an amount sufficient substantially to exalt the plating rate of said bath and being selected from the group consisting of succinic acid and salts thereof; wherein the absolute concentration of hypophosphite ions in said bath expressed in mole/liter is within the range 0.15 to 1.20, the ratio between nickel ions and hypophosphite ions in said bath expressed in molar concentrations is within the range 0.25 to 1.60, and the initial pH of said bath is within the approximate range 4.0 to 7.0.

20. The process of chemically plating with nickel a body comprising an element selected from the group consisting of iron, cobalt, nickel, aluminum, copper, silver, gold, palladium and platinum, which comprises contacting said body with a bath comprising an aqueous solution of a nickel salt and a hypophosphite and a chelating agent selected from the group consisting of aminoacetic acid and salts thereof and an exalting additive selected from the group consisting of succinic acid and salts thereof, the ratio between nickel ions and hypophosphite ions in said bath being in the range 0.25 to 1.60, the absolute concentration of hypophosphite ions in said bath being in the range 0.15 to 1.20 mole/liter, the absolute concentration of aminoacetic acid ions in said bath being sufficient to chelate at least 100% of the nickel ions therein so as to impart to said bath a phosphite tolerance of at least about 1 mole/liter, and the absolute concentration of succinic acid ions in said bath being at least 0.04 mole/liter so as substantially to exalt the plating rate of said bath.

21. The process of chemically plating with nickel a body comprising an element selected from the group consisting of iron, cobalt, nickel, aluminum, copper, silver, gold, palladium and platinum, which comprises contacting said body with a hot bath comprising an aqueous solution of a nickel salt and a hypophosphite and a chelating agent selected from the group consisting of aminoacetic acid and salts thereof and an exalting additive selected from the group consisting of succinic acid and salts there-

of, the temperature of said bath being above 90° C. and the pH of said bath being in the range 4.0 to 7.0, the ratio between nickel ions and hypophosphite ions in said bath being in the range 0.25 to 1.60, the absolute concentration of hypophosphite ions in said bath being in the range 0.15 to 1.20 moles/liter, the absolute concentration of aminoacetic acid ions in said bath being sufficient to chelate at least 100% of the nickel ions therein so as to impart to said bath a phosphite tolerance of at least about 1 mole/liter, and the absolute concentration of succinic acid ions in said bath being at least 0.04 mole/liter so as substantially to exalt the plating rate of said bath.

22. A bath for the chemical plating of a catalytic material with nickel comprising an aqueous solution of a nickel salt, a hypophosphite, a chelating agent, and a separate and different chemical type exalting additive; said agent being present in an amount sufficient to chelate at least 100% of the nickel ions in said bath so as to impart thereto a phosphite tolerance of at least about 1 mole/liter and having the general formula:



where: R is an aliphatic radical, X is a functional group containing a dissociable hydrogen atom and selected from the class consisting of:



and Y is a functional group containing a negative atom acting as a center of coordination and selected from the class consisting of:



and wherein the functional groups X and Y are in alpha or beta positions to each other; said additive being present in an amount sufficient substantially to exalt the plating rate of said bath and being selected from the group consisting of simple short chain saturated aliphatic monocarboxylic acids including 3 to 5 carbon atoms and salts thereof, simple short chain saturated aliphatic dicarboxylic acids including 3 to 6 carbon atoms and salts thereof, and short chain aliphatic aminocarboxylic acids and salts thereof; wherein the absolute concentration of hypophosphite ions in said bath expressed in mole/liter is within the range 0.15 to 1.20, the ratio between nickel ions and hypophosphite ions in said bath expressed in molar concentrations is within the range 0.25 to 1.60, and the initial pH of said bath is within the approximate range 4.0 to 11.0.

23. A bath for the chemical plating of a catalytic material with nickel comprising an aqueous solution of a nickel salt, a hypophosphite, a chelating agent, and a separate and different chemical type exalting additive; said agent being present in an amount sufficient to chelate at least 100% of the nickel ions in said bath so as to impart thereto a phosphite tolerance of at least about 1 mole/liter and being selected from the group consisting of lactic acid and salts thereof; said additive being present in an amount sufficient substantially to exalt the plating rate of said bath and being selected from the group consisting of succinic acids and salts thereof; wherein the absolute concentration of hypophosphite ions in said bath expressed in mole/liter is within the range 0.15 to 1.20, the ratio between nickel ions and hypophosphite ions in said bath expressed in molar concentrations is within the range 0.25 to 1.60, and the initial pH of said bath is within the approximate range 4.0 to 7.0.

24. A bath for the chemical plating of a catalytic material with nickel comprising an aqueous solution of a nickel salt, a hypophosphite, a chelating agent, and a separate and different chemical type exalting additive; said agent being present in an amount sufficient to chelate at least 100% of the nickel ions in said bath so as to impart thereto a phosphite tolerance of at least about 1 mole/liter

and being selected from the group consisting of malic acids and salts thereof; said additive being present in an amount sufficient substantially to exalt the plating rate of said bath and being selected from the group consisting of succinic acid and salts thereof; wherein the absolute concentration of hypophosphite ions in said bath expressed in mole/liter is within the range 0.15 to 1.20, the ratio between nickel ions and hypophosphite ions in said bath expressed in molar concentrations is within the range 0.25 to 1.60, and the initial pH of said bath is within the approximate range 4.0 to 7.0.

25. A bath for the chemical plating of a catalytic material with nickel comprising an aqueous solution of a nickel salt, a hypophosphite, a chelating agent, and a separate and different chemical type exalting additive; said agent being present in an amount sufficient to chelate at least 100% of the nickel ions in said bath so as to impart thereto a phosphite tolerance of at least about 1 mole/liter and being selected from the group consisting of malic acid and salts thereof; said additive being present in an amount sufficient substantially to exalt the plating rate of said bath and being selected from the group consisting of aminoacetic acid and salts thereof; wherein the absolute concentration of hypophosphite ions in said bath expressed in mole/liter is within the range 0.15 to 1.20, the ratio between nickel ions and hypophosphite ions in said bath expressed in molar concentrations is within the range 0.25 to 1.60, and the initial pH of said bath is within the approximate range 4.3 to 9.5.

26. A bath for the chemical plating of a catalytic material with nickel comprising an aqueous solution of a nickel salt, a hypophosphite, a chelating agent, and a separate and different chemical type exalting additive; said agent being present in an amount sufficient to chelate at least 100% of the nickel ions in said bath so as to impart thereto a phosphite tolerance of at least about 1 mole/liter and being selected from the group consisting of aminoacetic acid and salts thereof; said additive being present in an amount sufficient substantially to exalt the plating rate of said bath and being selected from the group consisting of succinic acid and salts thereof; wherein the absolute concentration of hypophosphite ions in said bath expressed in mole/liter is within the range 0.15 to 1.20, the ratio between nickel ions and hypophosphite ions in said bath expressed in molar concentrations is within the range 0.25 to 1.60, and the initial pH of said bath is within the approximate range 4.0 to 7.0.

27. The process of chemically plating with nickel a body essentially comprising an element selected from the group consisting of iron, cobalt, nickel, aluminum, copper, silver, gold, palladium and platinum, which comprises contacting said body with a bath comprising an aqueous solution of nickel ions, hypophosphite ions, lactic ions and succinate ions, wherein the absolute concentration of hypophosphite ions in said bath expressed in mole/liter is within the range 0.15 to 1.20, the ratio between nickel ions and hypophosphite ions in said bath expressed in molar concentrations is within the range 0.25 to 1.60, the absolute concentration of lactic ions in said bath expressed in mole/liter is at least about 0.2 so as to impart to said bath a phosphite tolerance of at least about 1 mole/liter and the absolute concentration of succinate ions in said bath expressed in mole/liter is at least about 0.06 so as substantially to exalt the plating rate of said bath.

28. The process of chemically plating with nickel a body essentially comprising an element selected from the group consisting of iron, cobalt, nickel, aluminum, copper, silver, gold, palladium and platinum, which comprises contacting said body with a bath comprising an aqueous solution of nickel ions, hypophosphite ions, a chelating agent, and a separate and different chemical type exalting additive; said agent being present in an amount sufficient to chelate at least 100% of the nickel ions in said bath so as to impart thereto a phosphite tolerance of at least about

1 mole/liter and being selected from the class consisting of alkyl and alkynol amines; said additive being present in an amount sufficient substantially to exalt the plating rate of said bath and being selected from the class consisting of carboxylic acids and salts thereof; wherein the absolute concentration of hypophosphite ions in said bath expressed in mole/liter is within the range 0.15 to 1.20, the ratio between nickel ions and hypophosphite ions in said bath expressed in molar concentrations is within the range 0.25 to 1.60, and the initial pH of said bath is within the approximate range 4.0 to 11.0.

29. A bath for the chemical plating of a catalytic material with nickel comprising an aqueous solution of a nickel salt, a hypophosphite, a chelating agent, and a separate and different chemical type exalting additive; said agent being present in an amount sufficient to chelate at least 100% of the nickel ions in said bath so as to impart thereto a phosphite tolerance of at least about 1

5

10

mole/liter and being selected from the class consisting of alkyl and alkynol amines; said additive being present in an amount sufficient substantially to exalt the plating rate of said bath and being selected from the class consisting of carboxylic acids and salts thereof; wherein the absolute concentration of hypophosphite ions in said bath expressed in mole/liter is within the range 0.15 to 1.20, the ratio between nickel ions and hypophosphite ions in said bath expressed in molar concentrations is within the range 0.25 to 1.60, and the initial pH of said bath is within the approximate range 4.0 to 11.0.

## References Cited in the file of this patent

## UNITED STATES PATENTS

- 2,532,283 Brenner et al. Dec. 5, 1950  
 2,658,842 Gutzeit et al. Nov. 10, 1953